

J. E. BLOOM.

# PROCESS AND APPARATUS FOR THE ELECTRICAL UTILIZATION OF MOLTEN SLAGS.

APPLICATION FILED MAY 3, 1920.

1,377,554.

Patented May 10, 1921.



**INVENTOR**

# UNITED STATES PATENT OFFICE.

JACOB E. BLOOM, OF BROOKLYN, NEW YORK.

## PROCESS AND APPARATUS FOR THE ELECTRICAL UTILIZATION OF MOLTEN SLAGS.

1,377,554.

Specification of Letters Patent. Patented May 10, 1921.

Application filed May 3, 1920. Serial No. 378,665.

To all whom it may concern:

Be it known that I, JACOB E. BLOOM, a citizen of the United States, residing at Brooklyn, city and State of New York, have invented certain new and useful Improvements in Processes and Apparatus for the Electrical Utilization of Molten Slags, of which the following is a specification.

This invention relates to the mixing or 10 compounding of hot molten slags from metallurgical smelters, converters, furnaces or the like, with other materials; under insulated conditions; and is illustrated herein by the manufacture of fertilizers; and 15 has for its object, the utilization (in effecting and activating the compoundings,) of the electrical and catalytic properties and qualities developed by the high heat of the molten slags while hot and of the hot gases 20 and emanations from the smelters, etc., and in and for the purpose of the recovery or extraction or the like, of values from or in the materials or the mixtures or emanations therefrom, and thereby obtaining products 25 of improved quality and increased amount, and with saving of cost of fuel. Other objects are set forth in the body of the specification and in the claims.

This invention embodies improvements 30 upon the apparatus parts of my U. S. Patents Nos. 1,338,352 and 1,338,353 dated April 27, 1920, and of my application for Patent, Serial Number 356708, filed February 6th, 1920, the latter for electrical treatments in 35 the compounding of solids with gases, etc., including fertilizers; and in which is described the theory and science of heat-emitted electrons, *i. e.*, of positive or negative electrons or both, emitted from highly heat-40 ed particles or bodies; and I therein describe my improved means of earthing or neutralizing and utilizing such emitted electrons of one sign only, and thereby leaving a charge of electrons of opposite sign, 45 upon the particles or solids and utilized in the compounding thereof; and said methods and means are improved upon, in this invention, wherein in lieu of an exterior costly source of heat, I use the high heat of molten 50 slags, a waste product, without cost for heat, to attain emissions of electrons from suitable materials, advantageously duly brought into contact with the molten slags and whereupon I duly earth, or neutralize or 55 charge other particles with the heat-emitted electrons of one sign only, leaving the op-

posite electrons or charge upon the particle, and thereby accelerating or activating its compounding with an oppositely charged or neutral particle with which it contacts under insulated conditions. And herein, I advantageously do not use or require high electric energy from exterior source, such as is used in the arc furnace and the like to attain the nitrogen fixation chemical reaction, but I use for reasons of economy, low energy, low voltage and amperage such being ample to perform the desired function, to wit: to earth the heat-emitted electrons of one sign only and simultaneously repel the opposite electrons; without such latter repulsion and insulation of the whole, such opposite electron would likewise be earthed, and which I prevent as herein described. In addition, I also utilize the well known catalytic property of incandescent bodies and surfaces, in activating desired reactions of contacting atoms, molecules or particles meeting on such incandescent surfaces.

By the term slags herein, I include the 80 vitreous matters, or cinders or scoria, as removed in the reduction of metals in sundry types of metallurgical furnaces, smelters, converters or the like; and I specifically illustrate and describe the invention in the 85 utilization of molten slags and the hot gaseous emanations from iron and steel furnaces and converters or the like, in the making of fertilizers; though it will be understood that the process is adaptable to other hot limpid 90 slags, and to attain products and values other than fertilizers.

As a process, generally stated, the invention consists in the mixing, fusing, dissolving and compounding under insulated conditions, a molten slag, from its source, with suitable materials, solids or gaseous, having values or desirable ingredients which are not naturally readily available, and which are modified and made immediately available by the process (as illustrated by mixing and fusing in hot slags, sundry siliceous or basic minerals comprising phosphorites or potash fertilizer ingredients not naturally in available form as fertilizers, but 95 which become readily available under ordinary soil conditions upon due compounding with the molten slags as described); and during the mixing, the process further consists, in the earthing or otherwise neutralizing from the mixture, the heat-emitted electrons of one sign only; and thereafter duly 100 105 110

- and suitably recovering values from the resulting mixture or emanations therefrom, or otherwise utilizing the whole, as upon due cooling and pulverizing for fertilizer use; 5 and such recovery of values, includes the due leaching from the slag mixture, of sundry soluble compounds made available therein, and the due recovery from the solution by evaporation; and including the recovery of 10 values from vapors, gases, fumes, dusts and the like passing off from the mixtures due to the heat thereof; and including the recovery of metals, including precious metals, from the fused mixture, which are freed by 15 the heat and separated by gravity or centrifugal force, from the slags.

As an additional step in some cases, I advantageously duly blow into and through the slag mixture under insulated conditions, 20 hot air or the hot waste gases, either with or without due purification, from the smelter stack, or converter or the like, advantageously ionized; and in the method now pursued in blowing hot air through steel 25 converters or the like; and advantageously electrified with one sign only, as described in my said Serial No. 356708; and thereupon, duly recover from the escaping gases, vapors, fumes and dust, the values, to wit: 30 gaseous reaction and other compounds, after due cooling and condensation, flocculation or the like.

I advantageously apply the process in mixing in the molten slag as taken hot from 35 its source, suitable materials in finely pulverized or comminuted form, which are readily fusible at the temperature of the slag, and which will result in chemical reactions or molecular associations or electrical adsorptions or the like compoundings when 40 fused, in a manner analogous to dissolving and compounding in liquids, and which compounds can, if desired, be duly recovered, separated from the slag, by a wet process 45 as by leaching and evaporation and crystallization, or by a dry process as by vaporization, sublimation, cooling, condensing, flocculation or the like. As an alternative process, in some cases, where two or more 50 different materials are to be treated to extract values, therefrom, in lieu of simultaneously treating same together, I duly treat the same separately by the method above described, in separate batches of molten 55 slags; and thereafter mix and compound together the said separate mixed batches, in substantially the same method; and likewise the vapors or gases from the separate batches, oppositely electrified. 60 As an alternative step in the process in extracting some values advantageously attainable at materially different temperatures, I conduct the process in a succession of steps, of conducting the above described 65 process at such different temperatures,

starting with the highest and continuing with the same or similar slag as it gradually cools, or utilizing well known means of cooling.

In the conduct of the process, I advantageously mix and fuse the materials successively, in the order of their several melting temperatures, *i.e.*, where all are mixed in the one batch of slag.

I advantageously use methods of feeding 75 the solid material comminuted; in thin spray-like or sheet-like form, or as a sand blast, previously warmed, to avoid chilling the molten slags; and duly agitating the mixture to attain intimate contact of particles, as with mechanical rabbles or stirring devices or with blasts of gases or otherwise. The temperature of slags from Bessemer steel converters, averages 1600 to 1800 degrees centigrade.

Most siliceous or basic minerals or rocks comprising fertilizers such as phosphorites or potash, readily fuse completely at 1310° to 1350° C. to a homogeneous mixture; and even at a lower temperature, as at or under 1050° C., there is an apparent near-fusion with the exception of a few minute crystals whose surfaces act as adsorbents in this process. This latter property is utilized where slags of lower temperature are used; 95 as for instance pig iron blast furnace slags which often have temperature of 1200° C. only.

It has been found, that under insulated conditions and high heat, inorganic substances begin to emit electrons at about 230° C., increasing materially at over 400° C.; and the emission is quite large at over 700° C.; and that phosphates of inorganic substances at high temperatures, emit generally 105 only positive electrons, and the atoms or particles from which these heat emissions emanate, are then negatively charged; and chlorides of inorganic substances likewise; and conversely, the oxides of inorganic substances at high temperatures emit generally 110 only negative electrons, and the particles are left positively charged,—and especially so, the alkali oxides, also the alkali metals and alloys; and the nitrates of inorganic substances at high temperatures, emit only 115 positive electrons until converted into oxides, after which only negative electrons are emitted. Again, the chemical reaction between gases and alkali oxides give rise to 120 emissions of negative electrons. The kind of emissions is readily determined by well known methods. Again, in some cases, at high temperature, both positive and negative electrons are emitted, notably with some 125 gases. The positive electrons liberated or emitted by the hot bodies, are associated with mass, or are structures of atomic or molecular dimensions; but not so the negative electrons, which are the same from all materials. 130

In my process, I utilize said electrical conditions or properties or charges, both as regards the solids and gases, and compounds in solution or in disperse state in the molten slags or mixtures, and also the emanations therefrom, some of which latter take up or combine with and carry off the heat emitted electrons, and thereby become electrified accordingly, either positive or negative; and I effect compoundings electrically, including chemical reactions, molecular associations and adsorptions, advantageously by the contact in the molten slags of the oppositely electrified solvates or dispersoids or the like, atoms, molecules or particles; and also of the oppositely charged emanations in the mixtures and after leaving the mixtures in the form of vapors, gases, fumes or the like; all under insulated conditions.

By the term emanations, I include, vapors, gases, fumes, dust or the like, formed by or in or escaping from the hot mixtures. By the term "oppositely electrified," I include cases where one of the contacting particles only is electrified, the other being neutral. By the term "extracting the values," I mean the duly obtaining from the mixtures, or materials, or from the emanations, any of the compounds or elements desired or of value, and in available form.

The composition of slags, ores, fluxes and the like, is not uniform, no two slags being alike; and for the same reasons, no exact electrical actions can be forecast, and must be empirically determined from successive results under same conditions, at the same plant, with the same materials mixed with slags from same origin.

By the alternative term "or neutralizing," *i. e.*, "earthing or neutralizing," I mean, where the heat emitted electrons from the molten mixture, or the like, in lieu of being electrically led to ground as through a ground wire of the unipolar contact and earthing apparatus as described in my said application, Serial No. 356,708, are neutralized and utilized by and upon meeting and being taken up by another molecule or ion, or atom or particle, and which is thereby electrified positive or negative, or which may be neutral or oppositely electrified, and which in latter case, may become neutralized; and such may be a solid or may be a gas or the like in the mixture, forcibly blown or otherwise brought into contact therewith by agitation. In some applications of the process, I electrify the gases prior to blowing same through the molten mixtures, with one sign only, the opposite to the prevailing sign of the mixture, or the latter may be neutral; and vice versa. The gases as led from the throat of a smelter or converter, or the like, generally have a temperature of about 750° C., and are readily ionized and electrified with one sign only without additional heating; as described and used in said Serial No. 356,708. And likewise as regards the hot emanations, gases, vapors, etc., from two different batches of slag mixtures, such are readily ionized and electrified with one sign only, opposite to each other, separately, and then brought together under insulated conditions, resulting in gaseous compounds of value, recovered as indicated, and having increased density and stability and diminished hygroscopicity. By increased density and stability, I mean increased as compared with like or analogous compounds formed or made by any process without the electrical process herein described; and by diminished hygroscopicity, I mean diminished as compared with the hygroscopic property of a like compound prepared by any process without the electrical process or steps herein described.

Where neutralization of the heat emitted electron occurs, as above described, and which is apt to occur when two different materials are fused or treated in the same batch of molten slag, such as phosphates emitting positive and alkalies emitting negative electrons, then the above unipolar contact and earthing apparatus is not used, and is cut out by opening the circuit breaking switch. The time of so doing is advantageously determined empirically starting with about twenty minutes agitation; or can be approximately pre-determined, by analysis and calculation of the amounts of said different components in the batch. But, it will be understood that the process is conducted under insulated conditions, the apparatus being supported on insulators. In the process, with some materials, as for instance those comprising potash, the latter or salts thereof, can be advantageously volatilized at lower temperatures, *i. e.*, lower than the original slag temperatures, at 500° C. to 800° C.; and slags should be cooled to such latter temperatures if it is desired to recover most of the potash in available state from a mixture with the potash materials, especially if there be in the slag a material per cent. of silica, which fixes the potash in a non-available state.

Again, as a step in the process, advantageously with low temperature slags, it is advantageous to add iron, hematite, or manganese dioxide ore, about 7% of each or both, to impart fluidity to the mixtures at the lower temperature; and such is often advantageous at the higher temperatures; and the addition of other materials, in granulated or pulverized form or as gases, will suggest itself to the chemist and metallurgist, to effect desirable compoundings of values to be recovered as above indicated, and from divers and other materials.

In the making of slag fertilizers with

this process, I advantageously add to the mixtures hereinafter described, manganese dioxide, or manganese ore, or manganeseiferous iron ore, or the like, in predetermined amount to attain advantageously not over 8% of manganese in the slag fertilizer product, not only to increase the fluidity of the molten mixture, but also as an additional fertilizer constituent in the product, serving as an activator in the plant food for which the fertilizer is used, and also when consumed as a constituent of such plant food, serving a useful function as an activator in the assimilative processes in the body or animal system.

As an alternative or additional step of or in the process, generally stated, the invention consists in the suitably collecting, blowing under regulable pressure, and mixing, under insulated conditions, the hot gases and emanations from the furnace or the like source of the molten slags, into and through mixtures of the molten slags with materials having values; and into contact with other gases, or gases and vapors, or the like, for due compounding therewith, and the recovery of values therefrom; or into contact with materials having values, which are also advantageously heated by convection of heat from molten slags; and the said hot furnace gases and emanations or the like, before the said mixing thereof, being advantageously electrified with one sign only, by the due earthing therefrom of the heat-emitted electrons of opposite sign only.

And likewise as regards electrically utilizing the hot vapors, gases and emanations arising from the molten slag mixtures. All such emanations from furnaces or the like, as also the same from molten slag mixtures, as also from mixtures of materials treated as herein described, carry ionized gases, and particles carrying negative or positive electrons or both, and from which a very large portion of electrons of one sign are readily earthed as described, leaving the particles electrified with opposite sign; and the subsequent compounding thereof with other neutral or oppositely electrified ions or atoms or molecules or colloids or particles is accelerated, with resulting compounds of increased density and stability.

The temperature of furnace gases, often exceeding 750° C., is sufficiently high to cause other and neutral particles with which the hot emanations contact as described, to also thereby become heated sufficiently high, to emit electrons, some of which are earthed or neutralized, leaving them electrified, and thereby further facilitating the desired combinations, and ensuing recovery of values.

As an apparatus, the invention, generally stated, comprises a suitable mixing cham-

ber of a vessel such as a slag pot or a retort, or converter, or slag-hearth, or tilting slag-car, or a rotatory puddling machine (mechanical, or rocking or oscillating), or hearth of a smelting furnace or like the by-product coke oven with stirrer, or the like, with chamber lining of conductor refractory substance, with insulator supports, with carbon or graphite brick or the like, back of the conductor refractory lining of the chamber, with hot limpid slags therein; with means of intermittently passing into the chamber, hot molten slags, and previously heated comminuted materials to be fused and mixed with the molten slags therein, with means of agitating and stirring the mixture advantageously with a graphite stirrer or the like; with means as described in Serial No. 356,708 of electrically earthing from the mixture, during the mixing, the heat emitted electrons of one sign only, or otherwise neutralizing such electrons, and retaining and repulsing into the mixture the electrons of opposite sign; with means of withdrawing the mixtures from the chamber; and advantageously, with means of blowing hot air, or waste gases from the source or furnace producing the said molten slags, or the like, through suitable twayers, into and through the molten mixtures in said chamber; with means of suitably collecting the emanations, gases, vapors, fumes, dusts or the like, escaping from the said chamber, into suitable conduits, chambers, flues, condensers, coils or the like; all under insulated conditions; and with means of recovering values from such emanations; with means for recovering values from the slag mixture; with means of pulverizing the remaining slag residue mixture after the due withdrawal from said chamber. By the term pulverizing slags, I include granulating, as by means of pouring the hot mixtures into a well of water, as at present; also means of making a pumaceous mass thereof as by spraying same with blasts of hot gases; and with means of subsequently or simultaneously cooling, and means of then grinding, or of then leaching to extract values from the more friable mass; or the like.

As an alternative apparatus, where two or more different materials, having different values, such as the phosphate and the alkali rocks, are to be treated in molten slags, then in lieu of the one apparatus aforesaid, I advantageously provide and use as described, two or more thereof; that is, the apparatus comprises, a separate electrical mixing unit, (substantially as above described for electrically utilizing one batch of molten slag only, for one or more materials mixed in the one batch of slag, and which I hereinafter call an "electrical mixing unit"), separate for the due mixing and treating 130

of each such different material, and separate means for collecting the emanations from each mixing chamber; and with means, similar to the said unit, of suitably enlarged 5 capacity, of similarly mixing and treating in the one chamber, such two batches together; or more than two batches; and advantageously with means to likewise bring together and duly mix the two emanations 10 from the separate units; or more than two; all under insulated conditions. And with means of recovering values from the emanations, separately or together; and with means of recovering values separately from 15 the remainder of each batch of slag mixture or from the single united mixture remaining from all the batches of slag mixtures; and with means of utilizing the latter thereafter, as for cements, or brick or otherwise; 20 or as fertilizer, when the fertilizer elements have not been entirely removed or emanated and recovered therefrom.

As an alternative apparatus, where two different materials having different kinds of 25 values are to be advantageously treated at materially different temperatures to recover values therefrom in increased amount, the apparatus comprises two separate electrical slag-mixing units with hot molten slags at 30 about the different temperatures; with means of cooling the slags accordingly before or during the mixing with the material to be mixed and treated at the lower temperature; such cooling means to comprise attemperating coils surrounding chambers and conduits to utilize the waste heats for steam making and heating materials before mixing with slags, etc.; or steel-jacketed spacings surrounding the mixing chamber 35 40 with refrigerating fluids flowing therethrough;—or with means of blowing cold gases or air through the mixture; or advantageously cooling by mixing and fusing in the molten slags at the higher temperature necessary to fuse the matrix, the material holding the value to be extracted or recovered, though there may thereby be a loss 45 of some of the desired value. This latter means of cooling, is advantageously pursued 50 also where only the one batch of slags, or one material only is treated, in order to insure limpidity of the slag mixture, and due fusion of the material, and the freeing of the values or the major portion thereof; 55 and to attain such fusion or freeing of values, an additional fluxing substance may be duly added to the mix, not only to act as a flux, but also as a harmless cooling agent to attain in the mix a desired lower temperature.

Well known means are duly provided, for determining the temperatures from time to time, of the slag mixtures, and also of the emanations of emanations; and with means of regulating and controlling the temperatures

and pressures of the latter in the several mixing and recovering flues, chambers, coils and accessory apparatus.

I advantageously cool the hot emanations, gases and the like, by passing same from 70 the mixing chamber to the recovery apparatus, or from the latter, through suitable flues or the like, surrounded by suitable receptacle for holding and thereby warming the materials to be subsequently mixed with 75 the slags. And in the absence of such emanations recovery apparatus, I similarly utilize the hot slags or the slag mixtures, advantageously in the desired cooling thereof, to warm suitable inclosing or surrounding 80 receptacles for holding and heating the materials to be mixed, and in order to avoid undue chilling of the slags upon first contacting with the materials, and to attain a more homogeneous chilling or cooling of the 85 whole mass.

The apparatus advantageously provides and includes suitable means of similarly electrically treating, and extracting the values from, the hot emanations from the 90 admixtures of the molten slags and materials fused therein, comprising insulated means for collecting the emanations from the mixing chamber into and through a suitable electric earthing conduit lined with 95 refractory conductor substances, and thence into suitable flues, and chambers for the recovery or precipitation of fumes and dusts or the like, as in metallurgical smelting practices, or as practised in the recovery of 100 values in and from by-product coking ovens, or other systems of recovering values as heretofore indicated; with insulator supports for the apparatus holding or conveying or treating the gases; with means of 105 earthing or neutralizing the electrons of one sign only, in the emanations, in passing through the earthing conduit, duly therein provided with the unipolar contact and earthing apparatus of Serial No. 356,708; 110 and thereby the emanations are charged with one sign only by the earthing of heat emitted electrons of the opposite sign only, and the particles carrying the one kind of charges, are thereafter more readily compounded with neutral or oppositely charged other particles for the contacting with which, means are duly provided in and by ensuing flues, chambers, coils and the like, 115 all on insulator supports, of the suitable 120 recovery apparatus, and including precipitation, flocculation and the like effect, as with fume or dust particles carrying such charges or electrons, upon striking and contacting with duly interposed baffles, plate 125 or wire screens or the like, on insulator supports, or advantageously oppositely electrified, that is by means of a similar unipolar contact earthing apparatus; with means of collecting the precipitations upon and from 130

such baffles. And similar means are provided for the unipolar electrification of a second or other stream of emanations from another batch of slag mixtures, suitable for 5 compounding with the aforesaid emanations, and with sign opposite to the latter; and with means of suitably bringing together and mixing, in a neutral conduit, flue, chamber, coils or the like on insulator 10 supports, the two oppositely charged streams of emanations; with suitable means for recovery of values from the combined streams.

And advantageously, where the materials mixed with the molten slags, comprise 15 metals, especially precious metals, which do not volatilize at the temperature of the slags, and which are heavier than the slags, whose specific gravity averages about 2.6, and which metals or mattes can therefore 20 be separated by gravity or centrifugals after being melted and freed by the heat of the slags,—then the apparatus further comprises a suitable molten-metal receiving chamber or receptacle, suitably connected 25 with the mixing chamber, with means of passage of the metal from the mixture thereto, when duly separated advantageously by quiescence and gravity, and the earthing of all electrification from the mixture and removing insulated conditions.

And advantageously, as an alternative means, where the system of twyers and blowers for injecting gases through the slag mixtures are not available, the apparatus 35 includes, for the due collection and transportation of the emanations from the mixing chamber, a suitable blower or suction means, in connection with the conduit and flues for the emanations, to duly propel the 40 same therethrough, in addition to the diffusion and expansive force of the hot gases.

And advantageously, where only a slag pot or slag tilting car or the like vessel is available as a mixer, the apparatus includes 45 a mechanical stirrer advantageously of pure graphite or lined therewith, or like the mechanical rabble of an iron mechanical pudder, of a conductor or metal or alloy material of far greater melting point than the 50 slag temperature, and advantageously with means of cooling the rabble like water-cooled electrodes, and with an insulator handle or dielectric refractory cover of the handle to enable the due stirring of the 55 mixture under insulated conditions, with insulator supports of the vessel; and such rabble is advantageously a hollow cylinder with suitable means for blowing and injecting hot air or gases or pulverized materials therethrough and into the molten slags or mixture simultaneously while stirring the mixture with the rabble and with the above unipolar contact and earthing device electrically connected to the rabble.

65 The apparatus advantageously includes

suitable means of feeding the materials to be mixed and fused in the molten slags, in pulverized form, duly warmed, and in thin streams, through a feed hopper in top or sides of chamber, with simultaneous agitation, either by mechanical stirrers or by due tilting or shaking of the vessel or the like, or by suitable injecting of the powders by a twyer injector with and by the simultaneous injection of hot gases, by means similar to 70 the like twyers and apparatus for blowing hot gases into and through blast furnaces or the like; or as described in my Serial No. 356,708.

Where the available slag mixing vessel 80 is of the type of a by-product coke oven, with a machine operated stirrer, the apparatus advantageously includes such-like stirrer in combination with the above unipolar contact and earthing apparatus electrically connected with the stirrer, and advantageously with a conductor refractory lining, and adjusted to earth the freed electrons of one sign only, upon contacting therewith during the agitation with the 90 stirrer, and simultaneously repulsing the opposite electrons or particles oppositely charged, and which latter are thereby utilized in ensuing compounding with other oppositely charged or neutral particle. Refractory lining for such ovens or other slag mixing chambers is advantageously made of a conductor substance like a carbon electrode or a graphite brick or a cement compounded of graphite and of basic oxids, lime or magnesia or dolomite or fluorspar or the like admixtures, *i. e.*, of some of the fluxes elsewhere herein stated as advantageous to mix with the slags and materials from which values are to be recovered, to serve the purpose therewith, analogous to the replaceable linings of basic slag furnaces, when corroded. Said lining is advantageously backed with a carbon filling between it and the outer wall or metal shell or the like, which filling and metal parts are likewise electrically connected with same unipol-earthing device as the conductor lining.

The apparatus advantageously includes, as where new smelters or open hearth furnaces, or converters or other source of slags including electric furnaces, are to be constructed insulator supports for such, as by means of one or more layers of massive porcelain, or stoneware, or lava or other solid insulator material, and advantageously water cooled are placed upon present foundation stones; and advantageously horizontally perforated to permit of the circulation therethrough of cold air or waters or the like; and otherwise conducting the smelting or the like operations under insulated conditions, including providing dielectric joints in connecting piping leading to the twyer and in the piping or conduits for the dis- 130

charge of the smelter gases; and in the feeding channels or ways for supplying of the components of the charge to the smelter; and the like; and in the slag run or cinder run 5 from the smelter or slag source, to the slag mixing chamber, I provide suitable conduit, preceded by a dielectric joint, and electrically connecting said conduit and its passing slags to earth the heat emitted electrons of 10 one sign only therefrom, through the above unipolar contacting and earthing apparatus; and likewise in the above smelter gas conduit; and in some cases in the hearth of the smelter or the like; and thereby obtaining 15 and using in my process, the slags electrified largely with one sign only, advantageously positive, and the gases ionized and electrified with opposite sign, advantageously negative. And advantageously lining 20 the smelter or converter or other source of the molten slags, with a refractory conductor substance or compound lining like that elsewhere herein described for the lining of slag mixing chambers, and similarly 25 electrically connecting the lining with a unipolar earthing device to earth the heat-emitted electrons of one sign only, advantageously the negative.

The apparatus includes the combination 30 of the above mixing chamber and mixtures, and agitators and the like, with the conductor refractory linings to attain extensive contacting surfaces for and with the earthing apparatus or device, or unipolar contacting 35 and earthing apparatus described in my aforesaid application Serial No. 356,708, and in my patents for electrical processes and apparatus, etc., Nos. 1,338,352, and 1,338,353, each dated April 27th, 1920, both filed September 30, 1919; i. e., using herein only the 40 contacting and earthing means, and disposing with the electrifier means which in this invention are practically the hot slags and hot gases and heat emitted electrons 45 therefrom.

In this invention, I advantageously use the direct current low voltage circuit, with means of earthing one pole thereof and bringing the other pole in contact with the 50 material being treated, under insulated conditions, as described, advantageously in said latter patents.

Though I may operate with a circuit of 55 low voltage and amperage continuously supplied, on account of the economy in cost thereof, yet where such cost is to be ignored, as where the waste heat of molten slags and furnace gases is utilized for steam making to drive steam engines to drive motor generators, dynamos and the like for creating the 60 electric circuits used in the unipolar contacting and earthing devices, then I may advantageously use currents of higher or medium voltage and of greater amperage; 65 and such latter, thus created and the herein

described unipolar contacting are advantageously used in the processes of said application No. 356,708 in the making of the fertilizer and other products therein described. And so likewise, in the present process, 70 where pulverized materials are to be blown into and mixed with sheets of falling molten slags from which electrons of one sign have been earthed, then I advantageously inject such pulverized materials previously electrified with sign like said earthed electron by 75 means of such greater current and as described in said 356,708. In the recovery or extracting of some values from the slag mixtures, advantageously after the principal 80 emanations have passed off therefrom, I advantageously provide means for an alternative or final granulating step in the process, to wit, in the granulating of the slag mixtures as by mechanical means such as by injecting or falling upon centrifugal revolving metallic cylinders or dispersers within 85 suitable chambers, or means of falling into a tower through a suitable metallic screen, or otherwise and in part, as is done in the 90 producing of cement from slags; in my improved step, I advantageously electrically connect such mechanical means, the centrifugal surfaces, or the screens or sieves and the 95 like contacting surfaces, and the jacketed walls of the chamber or tower, with my electrical earthing device as stated, for earthing heat emitted electrons of one sign only; and simultaneously injecting into the 100 suspended or falling granulated slags within the chamber or confined space, having insulator supports, streams of steam or vapors of a suitable solvent or disperse medium, suitable for dissolving any emanations, or some thereof, arising from the hot 105 grains of slag mixture suspended therein; and I further advantageously provide due means for collecting the said emanations from said granulated mixtures while suspended, and from the same upon their falling into a well of cold water or the like, and 110 duly transporting all such emanations, into the mixing conduits and flues for and with the above described emanations from the molten slag mixing chambers; and thereupon recovering the values from combined 115 emanations; and likewise from any solutions precipitated from the vapors in the chamber or tower. The granulated slag mixtures are thus made more porous, and 120 more readily give up their values in leaching operations, or other recovery processes.

As an alternative or additional step and 125 means for the recovery of values from the gases and emanations, and thereby largely purifying such before the final ejection of the waste gases into the exit chimney and atmosphere, I advantageously provide and insert in the final flue to the chimney, two successive conduit sections of piping, either 130

8  
 5 **U** or **S** shape or the like, of about the same cross section as the final flue, and with dielectric joints between the two sections and at the ends thereof, and on insulator supports, and with a filling in the bends of the **U**, of a loose bundle of metallic granules or wires or sieves or the like, with ample passageways for gases to pass therethrough; with each such bundle electrically connected  
 10 with my above unipolar electric contact and earthing device, the first to earth negative electrons only, and the second, positive only, or vice versa, with means of blowing or forcing the gases therethrough, with a door-way in the sections for withdrawing and replacing said bundles, and means of recovering values deposited upon said bundles or from the **U** sections; the detailed construction of such conduit sections being advantageously as described, in my said Serial No. 356,708, though herein, in most cases, the heating thereof will be dispensed with where the gases are still hot from the original slags.

25 By the term comminuted or pulverizing of materials for mixing into and with molten slags, I include and generally mean the coarse grinding thereof, the fineness thereof, varying with different materials, and the costs thereof; ordinarily 60 to 100 mesh is advantageous; I also include thereby, the decrepitation by heat, as with fluor-spar, which when coarsely ground or in small lumps, readily decrepitates in molten slags and therefore pulverizing is unnecessary. It is advantageous to first pass rocky material through a jaw crusher or the like to about one quarter inch size; then through crushing rolls to reduce to 20 to 60 mesh; 40 and in some cases, then grind or pulverize to pass through 100 mesh screen.

I provide means for suitably intermittently feeding the comminuted materials into the molten slags, as through a feed hopper or automatic door in roof of chamber, in such manner as to seal the opening against egress of gases or entrance of cold air; or injecting thin streams of comminuted materials against and into falling streams or 50 sheets of molten slags passing into the mixing chamber over wide edges or cascade steps within the walls inclosing the mixing chamber, or using other means of feeding and commingling the molten slags and comminuted materials more especially to attain a homogeneous heat admixture or, uniform high heat for vaporizing values from the materials, with or without the fusing thereof, as distinguished from the homogeneous 55 mixing of the atoms and molecules and the like of the slags and materials, which in some cases it is very difficult or impractical to effect on account of the high viscosity of some molten slags. Therefore, I advantageously provide the means indicated for

homogeneously spreading and utilizing the heat and heat-emitted electrons in the emanations, vaporizations or the like, especially where such occur at temperatures far below the fusing points of the materials.

I advantageously construct the walls of the slag mixing chamber, like the shell and walls of a steel converter, and with conductor refractory lining; and with conductor or carbon filling between the inner lining and outer metal shell or walls, and with like means for tipping, feeding and emptying same; and with like means of blowing hot gases therethrough, by means of suitable twyers. Or for open top vessels, I advantageously construct such, like the slag-hearth or the Spanish slag-hearth with twyers; and in all constructions, I provide insulator supports, and interior lining of a conductor refractory compound or a conductor brick like a graphite brick, or a compound cement of graphite or amorphous carbon advantageously bonded with refractories of basic nature, which when corroded will act as suitable admixtures or fluxes in the molten slag mixtures, like those elsewhere herein described. And such linings are electrically connected with a unipolar earthing device, like the stirrer connection, and likewise the metal shell or frame of the walls, to earth electrons of one sign only, as described.

As an alternative mixing chamber apparatus in lieu of a converter shell or the like, I provide a modification of the present by-product coking oven with mechanical stirrer, or the like; with insulator supports, and with the stirrers, and advantageously the chamber refractory conductor lining, and metal parts of walls electrically connected with my above unipolar earthing device; with additional means for feeding or pouring into same, the molten slags; and with analogous means for collecting the emanations.

I provide means of utilizing the dry methods of condensation in the treatment of large volumes of emanations, as in making slag fertilizers, by providing such means first, as are used in the separation of solid fumes, dust, etc., from smelter smokes, by cooling the gases, and by retardation of velocity through enlargement of flues, or change of direction or increase of surface friction; and further advantageously suspending numerous wire curtains in the flues, as at present, with the improvement of supporting such or the like, on insulator supports, and electrically connecting same with my above unipolar earthing device. Such flues are advantageously very long, as at present, and with the addition of insulator supports; and also of dielectric joints, at ends of sections in which said wires are suspended.

70

75

80

85

90

95

100

105

110

115

120

125

130

Means are duly provided for collecting and removing the fumes and dusts and flocculations and the like, precipitated in said flues; and further for the due recovery of 5 values therefrom, and also from the gases and remaining emanations duly carried beyond said depositions. Said emanations, in some cases, contain metallic values, as where such are in the materials mixed with the 10 molten slags, and volatilize therefrom; and again, where non-volatilizable, such may settle by gravity, and I provide means for the earthing of electrifications therefrom and for the settling and withdrawal thereof by 15 a suitable pipe connection with valve, from bottom of mixing chamber, in the form of a matte or metal or metallic compound, from which values are duly recovered.

As an alternative apparatus to utilize the 20 heat of molten slags, and the heat-emitted electrons, in some cases, where it is not desirable to mix the materials having values to be recovered, with the slags, I attain heat emitted electrons and ensuing recoveries of 25 values, by means of convection of the heat through an intervening solid conductor refractory plate or bowl or smelting furnace hearth, or crucible, or retort, or the like, or muffle or cupola furnace and with insulator supports, and which rests upon or 30 in the molten slag, and which retort or the like holds or supports the said materials, which are thus heated, deflagrated, or fused or the like, often with ensuing emanations 35 of gases, vapors, fumes and the like, together with heat emitted electrons from the materials or from the intervening hot infusible refractory plate; and the values are subsequently recovered from said emanations, 40 as also from the remainder of the materials in the bowl or the like, substantially as herein stated for and from the above slag mixtures; and for and with such, I provide and adapt like accessory means as 45 above described and with my unipolar contact and earthing device for earthing one kind of electrons and repulsing and retaining the opposite kind of electrons, as more fully described in my Serial No. 356,708,— 50 though it will be understood that the heat source therein stated, is replaced in this invention, by the molten slags. It will be understood, that I provide such retort-like furnace, duly set into a bath of molten slags in 55 a suitable slag pot, with means of separately introducing into the retort sundry materials in some cases, including gases, for due compounding, and with connections from the retort to condensers and the like; with means 60 of stirring or otherwise agitating the retort contents and of periodically emptying and refilling the retort; and with means of pouring the slags into the surrounding bath, and withdrawing same therefrom; and means of 65 tempering and insulator supports for

same. Most of the solids compounded with gases and sprays as described in said Serial No. 356,708, can be advantageously compounded in the above means, and methods, where economically available at or near the 70 source of the molten slags.

As a product, the invention generally stated, comprises a compound of values electrically recovered from or with a molten slag with other materials comprising values, 75 embodying and comprising compound of chemical reactions, and molecular associations, and electric adsorptions, and the like, whereof the compounded molecules and the like, have increased density and stability 80 and less hygroscopicity, meaning, as compared with similar products otherwise recovered or manufactured or obtained.

As a fertilizer product, generally stated, the invention comprises a pulverized electrically compounded slag with fertilizer 85 values of materials compounded or fused therein and therewith and thereby, embodying and comprising compound of fertilizer ingredients in available state, the com- 90 pounds comprising chemical reactions, molecular associations, and electrical adsorptions, and the like, and whereof the molecules and the like have increased density and stability 95 and decreased hygroscopicity; and in some 95 cases, distinguished by the elimination of deleterious components from the burnt product. Such fertilizer values include sundry soluble phosphates, and potash and nitrogen compounds, or either or any two thereof, 100 in the available forms desired, and also lime, and in some cases magnesia; and again, minor parts of soluble oxids of iron and advantageously of manganese or the like activator or catalytic assimilable element. 105

Again, in some products, as where the molten slags are duly mixed with materials comprising nitrogen, including gases including nitrogen fixed from air, or from smelter gases, or from cement making plants, 110 or from by-product coke ovens or the like, the product comprises such values in available form. Again, fertilizers are now made from basic slags, where the ores used contain phosphatic ingredients; but where the 115 latter are absent, as in most U. S. iron ores, and where only acid slags are obtainable, a product with phosphates is obtained by this process from the mixing of slags with phosphatic rocks, and having the above qualities or distinguishing characteristics. 120

As a product, the invention further comprises values recovered as described, including chemical compounds or molecular associations, or adsorption compounds of two 125 molecules or atoms or ions or particles or colloids or the like, from each of which, or one thereof, there have been removed or neutralized heat-emitted electrons of one sign only; or which have taken up a heat- 130

emitted electrons emitted from a neighboring particle; and which have thereby become electrified with one sign only, and opposite to each other; or one component being 5 electrified and the other neutral; all such prior to the compounding. And one such compound may thereupon further compound with a third atom or molecule or particle, or with a compound like unto itself, such 10 latter being oppositely electrified and the resulting compound being a molecular association. And all such compounds have increased density due to the electrical pressures in the compounding, which results 15 in increased stability, with diminished hygroscopicity. And likewise as regards the electrically combined adsorption compounds. In the molten slags, there are sundry colloids, electrically charged by the heat effects, while molten or suspended in the molten slags or in some cases, in the emanations; and including the sundry metal elements present from the metallic ores with 20 which the furnace or the like was charged; 25 and where such metals or mattes thereof are desired to be recovered, such may be electrically discharged by the described process, and the subsidence by gravity facilitated, and the values recovered in neutral state. I 30 attain my invention by the novel electrical apparatus in combination with sundry existing apparatus illustrated diagrammatically in the accompanying drawings, in which similar letters and numbers refer to similar parts; 35 but it will be understood, I do not restrict myself to the particular means described, other suitable apparatus being readily adaptable by a skilled engineer, with the addition of similarly combining therewith 40 the unipolar contacting and earthing means or device and with insulator supports and dielectric joints and the like to attain insulated conditions in the conduct of the process.

45 Figure 1 is a vertical section, in diagram of an open-top slag-mixer with insulator supports, with stirrer, in combination with an electrical unipolar earthing device. Fig. 2 is a diagram of a vertical section of a 50 furnace or other source of molten slags and hot gases, with effluent connections to three slag-mixers, with means of collecting gaseous emanations therefrom, and recovering values therefrom and from the slag-mixtures; with insulator supports of all apparatus; with unipolar earthing devices, whereof details are shown in Fig. 1. Fig. 3 is a 55 diagram of vertical section of a retort-like or closed-top mixer, set in a molten-slag 60 bath, with means of forcing hot gases through the mixer and contents, with stirrer operating in the mixer, with insulator supports, with unipolar earthing devices. Fig. 65 set in a hot-slag bath, with hollow stirring

rod and means of injecting hot gases into the mixer contents through stirrer, with insulator supports, with unipolar earthing device. Fig. 5 is a diagram in perspective of a furnace-slag-tap, with molten slag being 70 poured into a slag-run, (to or from a slag-mixer, not shown,) with insulator supports, with unipolar earthing device from the molten slags. Fig. 6 is a diagram of a perspective view of a slag-run, such as Fig. 75 5, combined with a slag-spreader, with means of blowing pulverized materials against the spreader while the slags are flowing thereover, and thence into a slag-mixer, with insulator supports, with unipolar earthing device. 80

In general, letter S indicates hot slags and mixtures; S<sup>1</sup>, etc., hot slag mixers; G, gas piping from mixers; P, electrifier conduits for gases and emanations; E E, the electrifier 85 earthing device; r, hot slag runs, or troughs; I, slag-inlets; L, lining of refractory conductor substance; C, cooling coils or for steam, or heating sands, etc.; T, twyers; R, rabble or any stirring device; D J, dielectric 90 joint; Y, insulator support; g, inlet port for powders into mixers.

Fig. 1 is a diagram of a vertical section of an open-top slag-mixing chamber S<sup>1</sup>; like the present slag-pot, or slag-tilting car, 95 or a slag-hearth, or the like, with insulator supports Y, with a mechanical stirrer R, with a conductor refractory lining L of said chamber S<sup>1</sup>, and whereof n represents an outer metal shell, and m is a filling of carbon, or like the walls of a steel converter, between n and L, and which stirrer has an insulator handle or cover to handle Y, and the said R and the said lining L and shell n of the chamber, being electrically connected to a unipolar earthing device, generally indicated by the letters E E, and fully described in my aforesaid patent application, and illustrated in part in Fig. 1, in which 100 D C G is a direct current generator or storage battery or other source of a direct current circuit, with pole-changer P C in the circuit, with one lead wire W' therefrom to earth, and the other lead wire w, to rabble or stirrer R and to contact lining L, and with voltmeter V' and ammeter A' and galvanometer not shown, and resistance R', and cut-out switch s, and clamp C E, (being a detachable clamp for attaching wire w to R and to L) in the said circuit and shown 110 in the wire w, and with the molten slag mixture S in the chamber S<sup>1</sup>, in contact with L and with R. It will be understood that by the letters E E, I also include the use of other analogous unipolar contacting 115 and earthing devices described in my above patent applications; and that any such, with a single chamber as above, constitutes a 120 slag mixing unit.

Fig. 2 is a diagram of vertical sections 125

of a combination of three several slag-mixing chambers or units: S<sup>1</sup>, S<sup>2</sup>, and S<sup>3</sup>, with closed top having inlet ports g for materials into the molten slags, and also having inlet conduits I for feeding molten slags falling from slag-runs r, from the slag source, to wit: a smelter, or open-hearth steel furnace, or a converter or the like Z; the slag-run r—being shown leading to S<sup>1</sup> holding a slag-mixture P, as of phosphorites; and slag-run r+ leading slags from Z to S<sup>2</sup> holding such as potash K mixture; and with slag-runs r<sup>1</sup> and r<sup>2</sup> leading slag mixtures from S<sup>1</sup> and S<sup>2</sup> respectively to the third mixing unit S<sup>3</sup>; and with twyers T<sup>1</sup>, and T<sup>2</sup>, and T<sup>3</sup> for blowing hot gases from the smelter or other source of waste gases, into and through said vessels S<sup>1</sup>, S<sup>2</sup>, and S<sup>3</sup> respectively, and into and through retort-like necks or conduits G<sup>1</sup>, and G<sup>2</sup> and G<sup>3</sup> respectively from S<sup>1</sup> and S<sup>2</sup> and S<sup>3</sup>, together with the hot vapors, gases and emanations therefrom,—all being duly continuously blown into gas-mixing conduits or apparatus G M,—and thence into suitable fume and dust and floccular precipitations collectors F; and thence into suitable gaseous and other recovery apparatus G C; and thence forcing the waste gases to purifier conduits P<sup>1</sup> and P<sup>2</sup> with metallic sieves or the like, a' and a' electrically earthed as shown; and thence to chimney A and the atmosphere, S G<sup>1</sup> and S G<sup>2</sup> and S G<sup>3</sup> are gas conduits leading the hot smelter gases or the like, to twyers T<sup>1</sup>, T<sup>2</sup> and T<sup>3</sup> respectively, with suitable blowers not shown, with regulable pressure. Insulator supports Y are shown for the sundry vessels and such are also used though not shown for the conduits, and connecting piping,—and which are also provided with dielectric joints D J, at points shown and elsewhere wherever it is essential to maintain operating under insulated conditions. At C C are cooling coils or the like for duly utilizing waste heats as for steam boilers or heating materials to be mixed with molten slags, or other heating purposes.

M' represents a receptacle below any mixer, as S<sup>2</sup>, for receiving molten metals or mattes, as of precious metals, settling in the molten mixtures by gravity and periodically allowed to fall into M' through a suitable exit pipe and dielectric joint connection from bottom of mixer, with cut-off valve in the exit pipe, not shown.

The unipolar earthing device E E, advantageously like that illustrated in Fig. 1, is duly electrically connected with the conductor refractory linings of the vessels and conduits at the points indicated diagrammatically in Fig. 2. It will be understood the said three units may be operated together, as stated, or each separately; and that means, not shown, are provided for

70 withdrawing the slag mixtures or residues from the chambers; and for the due recovery of values from such residues as also from the emanations either those from each mixing chamber separately or all together as indicated.

The slag-mixtures from S<sup>3</sup>, or the residues therefrom after the emanations therefrom have been allowed to pass off, if thus desired, are duly withdrawn from the bottom, 75 by opening suitable shut-off valves, not shown, and allowed to flow by gravity, through slag-run r<sup>3</sup>, into a granulating chamber and cold water pit W,—the slag-mixtures being advantageously sprayed by 80 being blown by a blast of cold air or some of the waste emanations from a branch S G<sup>5</sup> from G<sup>3</sup> by a twyer blast T<sup>4</sup>, so that the molten stream is first projected upon and is sprayed by falling upon the well-known 85 centrifugal or revolving cylinder W<sup>2</sup>, or using a cold-blast air injector W<sup>3</sup>, to so do,—and the falling grains and sprays while en route to the cold-water pit W<sup>4</sup>, are granulated and further in some cases made porous 90 by meeting a stream of gases or vapors or emanations injected through a twyer or injector T<sup>5</sup>; and the hot gases and vapors or the like are duly blown through W into exit pipe G<sup>4</sup>, and thence into F and ensuing 95 recovery apparatus. W and G<sup>4</sup>, are advantageously supported on insulators, not shown; and the granulating centrifugal W<sup>2</sup> electrically connected with E E, to earth negative electrons.

100 The waste heat from the emanations and gases and slag mixture prior to granulating the latter are used for heating the various materials prior to mixing with slags to avoid chilling the latter; also for making steam to drive dynamos and motors and the electric currents used in the process or for other lighting and power purposes, all by well known means not shown.

105 Fig. 3 is a diagram of a vertical section of a retort-like vessel or chamber V, the body or flask of which may be a long tube, or like a destructive distillation apparatus, with the chamber lined with conductor refractory lining, not shown with insulator 110 supports Y, advantageously with a stirrer R projecting into V for agitating mixtures of materials therein, with means of electrically connecting the stirrer and the lining E E, a unipolar earthing device; with inlet ports g for feeding materials M to be mixed and treated in the chamber; with inlet conduits I' for injecting gases or powders and gases into M; with dielectric joint D J, in conduit I', electrically connected with E E; 115 with neck or outlet pipe G<sup>5</sup> for emanations and gases from V and into suitable condensing and recovery apparatus; not shown, like the same indicated in Fig. 2; with an injector G J for injecting vapors or react- 120

125

- ing gases or the like into  $G^5$ , electrically connected with  $E E$ , analogous to and for like functions to similar injector  $G J$  of Fig. 2; and with means of attemperating  $M$ , not shown; with means of withdrawing  $M$  from  $V$ , not shown; with means of surrounding the flask or body of  $V$  or setting same in a bath of molten slag  $S$ , in a vessel  $S^4$  on insulator supports  $Y$ , and the vessel 10  $V$  also having insulator supports; and with means not shown of pouring molten slags  $S$  of high or low temperature, into  $S^4$ ; with cooling or attemperating coils  $C$  surrounding the vessel  $S^4$ , and exit conduit  $G^5$  and 15 the like, and simultaneously thereby using waste heat for generating steam for electric light and power purposes, including that utilized in  $E E$ , the unipolar contacting and earthing device. Similar coils  $C$ , or 20 the like means for utilizing the waste heats from molten slags, or from the smelter gases, or from the emanations described, are also shown and used in various parts of the apparatus of Fig. 2. It will be noted, that 25 Fig. 3, is an alternative form of apparatus, wherein the materials  $M$  having values to be recovered, are advantageously treated at lower temperatures than molten slags, or advantageously not mixed with molten slags, 30 but with heat-emitted electrons therefrom or from the highly heated metal frame of  $V$  in contact with the slags, or from the gases and emanations carrying electrons from prior contact thereof with molten slags of 35 the gases and emanations injected into  $M$  through  $I'$ , or in some cases, through the hollow rabble  $R$ . And likewise in Fig. 4.
- Fig. 4 is a diagram of a vertical section of an open-top kettle or the like,  $V^2$ , on insulator supports  $Y$ , with conductor refractory lining of the chamber, not shown, holding materials  $M$  in comminuted form, to be treated, and with stirrer  $R$ , with means not shown of blowing hot gases through  $R$ , with 40 means of setting the kettle  $V^2$  in a bath of molten slag  $S$ , in a slag-pot  $S^4$ , on insulator supports  $Y$ , with cooling coils  $C$  surrounding  $S^4$ , with  $R$  and conductor lining of  $V^2$ , electrically connected to  $E E$ .
- Fig. 5 is a diagram or perspective view 45 of a slag tap  $t$  from the source not shown, leading the molten slags  $S$  to a slag-run or trough  $r$ , on insulator supports  $Y$ , and provided with a conductor refractory lining  $L$ , and advantageously with cross-wise strips or low baffle plates or bundle of wires  $a$ , over which the slags flow, before passing by gravity into molten slag mixing chambers, not shown; and the said  $L$  and  $a$ , being 50 electrically connected to  $E E$ , a unipolar earthing device, to earth from the passing slags, electrons of one sign only, and whereby or whereupon the slags pass into the mixing chambers largely electrified with 55 positive sign. The slag-runs of Fig. 2, are

advantageously thus constructed. Such are termed electrifier slag-runs.

The conductor refractory linings for the above described electron contacting, to earth the heat-emitted electrons of one sign only, are made advantageously of amorphous carbon, such as charcoal or lamp-black or gas-retort coke or petroleum coke, with a binding material of waterglass or tar, and practically as now employed in making carbon mixtures for arc-electrodes or carbon battery plates or carbon brushes; and with the addition to the mixture, of acid or basic refractories, pulverized, of the same minerals, silica constituents or lime and magnesia, respectively, *i. e.*, similar to the fluxes or admixtures added to the molten slag mixtures herein described; when the latter is made basic, no acid lining should be used, that is no silica or the like is used in the 75 lining, but advantageously sundry basic minerals and advantageously oxids of  $K$  or of  $Na$  or of  $Mn$  or of  $Fe$ , that is oxids which are 80 advantageous in a fertilizer when such is being made by this process,—and which may 85 find their way into the slag mixtures when the lining is, in time corroded and disintegrated. In the latter event, the lining is 90 periodically renewed.

Where the lower slag temperatures are 95 used, as herein described, in some cases, a metal lining is advantageous, of good conductor metal, which will not fuse or melt or deteriorate at such temperature.

Fig. 6 is a diagram of a slag-spreader 100 plate  $r^6$ , advantageously provided to receive the slags  $S$  falling from slag-run  $r$  or the like, into a slag pot or slag mixer  $S I$ ; and while falling on such inclined plate  $r^6$ , the materials with values to be mixed with the slags, are injected in hot and sand-like form by suitable blasts through injectors 10 against the slags; the spreader plate being lined with a conductor refractory substance like slag-runs, and electrically connected with a unipolar earthing device  $E E$  to earth heat emitted electrons of one sign only.  $S^1$  may be either an open slag pot, or like Fig. 1, or a retort like chamber as in Fig. 2. Where the comminuted materials thus 110 injected into the thin streams of molten slags on the spreader, are phosphorites, the unipolar device  $E E$  is adjusted to earth positive only, both from the injectors 10, and the mixture  $S^1$ . In the preceding slag run, the 115 negative is earthed. On the spreader plate, and in the mixing chamber, the negatively charged phosphates combine with the positively charged lime and the like; forming calcium phosphates. Lime or magnesia or the like admixtures, are advantageously 120 similarly and separately projected, earthing the negative therefrom,—and so doing prior to injecting the phosphorites.

It will be understood, that the slag-runs 125

$r-$  and  $r+$  of Fig. 2 are like Fig. 5 in construction, and electrically connected with a uni-polar earthing device EE, to earth from the slags flowing therethrough only negative or only positive electrons respectively as shown; *i. e.*, the slags conveyed to  $S^1$ , in which phosphorites P are mixed and which give off positive electrons by high heat and thus become negatively charged, the flowing slags are advantageously positively charged by earthing negative heat-emitted electrons therefrom; and conversely, as regards the alkali materials K in slag mixture  $S^2$ , and the slags flowing in run-way  $r+$ . And likewise, as regards run-ways  $r^1$  and  $r^2$  which lead slag mixtures, from  $S^1$  and  $S^2$  respectively into  $S^3$  may be advantageously electrically connected to earth opposite electrons respectively, prior to mixing in  $S^3$ .

The operation of the apparatus is conducted as indicated in the description thereof, and of the process; and, in general tapping the slag tap t of the furnace; allowing the molten slags S to fall into slag-run  $r$ , contacting with baffles a therein connected with E E, adjusted to earth positive electrons if the slags be basic, with phosphorites, or negative for acid slags; thence allowing the slags to fall into slag pot  $S^1$  or the like of Fig. 1, or Fig. 2, and simultaneously feeding therein the comminuted material, and agitating the mixture with stirrer R of Fig. 1, or blast of hot gases Fig. 2, and adjusting the unipolar earthing device, to earth positive electrons if the materials comprise phosphorites or the like, and to earth negative electrons, if the materials comprise potash; that is to say, where the materials comprise particles whose heat-emitted electrons are mainly negative, as with alkalis, then the negative is earthed, as from  $S^2$ , leaving the particles charged positive; and conversely where the heat emitted electrons are largely positive, as with phosphoritic materials, then the positive electrons are earthed as from  $S^1$ , leaving the particles charged negative. Where both such  $S^1$  and  $S^2$  are simultaneously operated, the molten slag mixtures are then mixed in  $S^3$ , which has no earth connection; and being transported thereto over or in connecting slag-runs  $r^1$  and  $r^2$ , respectively, advantageously similarly earth connected like  $S^1$  and  $S^2$ .

The emanations from  $S^1$ , Fig. 1 escape into space, and are wasted; but in Fig. 2, such are shown, as indicated, duly led into conduit  $G^1$ , and meeting the emanations from  $S^2$ , via  $G^2$ , and emanations from  $S^3$  via  $G^3$ , and all together in conduit G M, and thence blown into fume and dust collectors F, and ensuing condensers C or other recovery apparatus and finally into the twin or consecutive adsorption conduits  $P^1$  and  $P^2$ , and thence to chimney A, to the atmosphere or

space at large and with unipolar earth connection as shown or described, from the conduits and recovery apparatus or the like.

In the conduct of the process and apparatus for making fertilizer products, I advantageously utilize hot molten acid slags, which, usually comprise no or very little phosphatic materials, with silicious or basic minerals comprising such phosphorites or phosphates, chiefly those with tricalcium phosphate; and which minerals are fusible in the molten slags; and likewise, advantageously separately sundry potash silicate rocks, such as "greensand" or glauconite; or the sericite slates; or the "leucite" rocks; or the like materials in crushed or coarsely comminuted or pulverized form; or I mix the finely ground mill-tailings containing potash salts or the silicates of potassium as now found in the dumps of wastes of sundry metallurgical plants; and I advantageously volatilize the potash salts as described for recovery of values, as in Fig. 2, and in addition to recovering the potash salts from the emanations, I also recover a material part of the remaining precious metal content whose specific gravity is greater than the slags or slag mixture, and as described. Or I mix with the molten slag mixtures of the above character, nitrate bearing earths or rocks which are now not utilized, on account of cost of recovery of nitrates with present processes; or I mix some of the nitrogen gases from by-product coking ovens or the like, or from and with the smelter gases, duly blown through the molten slag mixtures as described; or I mix some of the cyanamids or calcium nitrates or the like, described in my above Serial No. 356,708, advantageously while still hot from the original manufacture thereof. It will be understood, that the economic situation will largely govern the use of any such above materials, notably the costs of bringing the materials to the furnaces where the molten slags are produced, for due mixing therewith at the source, without additional consumption of fuel; and thereby utilize the present waste heat in the form of additional commercial by-products of the smelter or converter or the like.

In the operation of the process with molten slag mixtures, it is important to previously ascertain the average approximate composition or percentages of ingredients of the slags, and also of the materials to be mixed therewith, and thereupon the relative amounts of the materials and the slags, and either with or without additional suitable other admixtures such as lime or magnesia or dolomite or silica or the like, can be readily determined by the same general rules as adopted by the skilled metallurgist in determining like questions in mixing ores and fluxes in smelting operations. As a guide, the following authoritative quotations,

are adopted Technical Paper 187 of 1918, of the U. S. Bureau of Mines, page 17, states that the blast-furnace slag analysis average from 44% of pig-iron production, as follows: CaO 40.17%;  $Al_2O_3$  13.07%;  $SiO_2$  35.32%; and MgO 5.51%; CaS 3.87%; other oxids 2.06%.

"The percentage of the so-called "bases" is 51.61%, whereas the percentage of the "acids" is 48.39%." (Page 25): Average analyses of slag from furnace producing "basic" iron: CaO 44.34%;  $Al_2O_3$  11.84%;  $SiO_2$  35.97%. Again, the Carnegie Steel Co. of Pittsburg, Pa., reports the "chemical analyses of air-cooled blast furnace slags" from nine distant and different plants and localities, with composition as follows:

|                                  | Percentages.   |
|----------------------------------|----------------|
| 20 Silica-----                   | 31.53 to 36.72 |
| Alumina-----                     | 12.39 to 14.11 |
| Calcium oxid-----                | 38.75 to 45.8  |
| Magnesium oxid-----              | 1.62 to 19.43  |
| Iron oxid-----                   | 0.25 to 2.00   |
| 25 Sulfur in calcium sulfid----- | 0.89 to 1.29   |
| Sulfur in calcium sulfate-----   | 0.1 to 0.52    |

Basic slags from iron ores, which abound in Europe but not in the U. S., have been demonstrated by agriculturists to comprise the phosphates, duly abstracted from the ores, and to be contained in the slags as soil-soluble phosphates of lime and phosphates of magnesia; and generally as the tetra-basic-phosphate of lime or of magnesia, or of both. Such readily dissolve in water saturated with  $CO_2$  or in like soil conditions, forming an acid phosphate of lime, or of magnesia, the former like that found in the commercial superphosphates.

40 My electrical improvement enables the attaining of a similar composition of soil-soluble phosphates in slags from ores destitute of phosphorus or phosphates, by the due mixing with molten slags from such ores, or with acid slags, of materials comprising phosphorites or the like, together with basic elements where such are deficient, in the slags or the materials, such as lime or calcite, or magnesia, or dolomite, or the like 45 in ample calculated amount to combine with the phosphates present in order to form sundry phosphates of lime or phosphates of magnesia; and also silicates of lime or other base, wherever silica is in excess; 50 and for that a siliceous slag cannot so do, and is advantageously converted into the composition of or approximating a basic slag, by the admixtures indicated.

Mixtures of acid slags with phosphatic 60 limestone have heretofore been made by ordinary methods of mixing, but in most cases, though ample percentages of phosphoric acid were present, yet only a slight portion thereof, say one-tenth to two-tenths 65 was soluble in citric acid or soil condition

and which makes such commercially unprofitable, and due probably to the large excess of free uncombined silica and which latter defect is avoided by my electrical process, probably from the following cause.

Generally, lime CaO at the high temperature of the molten slags, emits negative electrons, and itself becomes positive. Silica  $SiO_2$  on the contrary (with its additional element of O), emits positive electrons, and itself becomes negative, and thereupon readily combines with the positive lime upon contacting therewith. And likewise, phosphoric acid  $P_2O_5$  with its excess of O, emits positive electrons and itself becomes negatively charged, and thereupon readily combines with the lime or the like base, and simultaneously repels the similarly charged silica.

One such acid slag from open hearth steel 85 furnace was found upon analysis to comprise percentages as follows: silica 50.26; lime CaO, 1%;  $F_2O$  32.80;  $MnO$  15.10. One such phosphatic limestone constituents comprised lime 51.54%; phosphoric acid 22.27%;  $CO_2$  90 17.20%; and  $SiO_2Al_2O_3$  8.99%.

It will be understood that no two slags even from the same source, and likewise no two such materials as said phosphatic limestone, analyze exactly alike; but a fair average based thereon can be assumed.

Quoting from "Separate No. 730 from Yearbook U. S. Department of Agriculture, 1917:"

"High-grade phosphorite or phosphate 100 rock, consists chiefly of tricalcium phosphate, commonly called bone phosphate of lime. The commercial grades range from 65 to 78% of this compound and contain as impurities, varying amounts of silica carbonates, fluorids and oxids or phosphates of iron, and aluminum." \* \* \*

"For producing soluble and available phosphates, without the use of sulfuric acid \* \* \* there are two general processes 110 \* \* \*. The first of these is based on the production of phosphate compounds which undergo ready decomposition under soil conditions. In this class is the phosphate of basic slag, a substance which is now universally recognized as a highly desirable phosphatic fertilizer." \* \* \*

"The other method of producing phosphoric acid, \* \* \* is based on the volatilization of this acid from its compounds, 120 and its subsequent collection. \* \* \* The general scheme consists in submitting an intimate mixture of phosphate rock and sand, with or without coke, to the action of a temperature sufficiently high, to drive off the phosphoric acid, and produce a slag consisting chiefly of silicate of lime. This slag contains most of the impurities originally present in the phosphate rock. The nearly pure phosphoric acid volatilized \* \* \* 130

absorbed in water, \* \* \* can then be used either for treating a second batch of phosphate rock and producing thereby double acid phosphate, or it may be neutralized 5 with ammonia, forming ammonium phosphate, one of the most concentrated fertilizers it is possible to produce. \* \* \* It renders possible the utilization of lower grades of phosphate unsuitable for treatment with sulfuric acid. Moreover, the product obtained is phosphoric acid in such a concentrated form that long railroad hauls would be commercially practicable."

Again, quoting from Bulletin No. 143 of 15 1914, U. S. Department of Agriculture, on "The production and fertilizer value of citric-soluble phosphoric acid and potash." "Composition of phosphatic limestone:  $P_2O_5$ , 20%; CaO, 37.1%;  $SiO_2$ , 32.4%; 20  $CO_2$ , 10.5%."

In the manufacture of the concentrated fertilizer, such as the above ammonium phosphate, I advantageously apply my aforesaid process and apparatus, advantageously as described for Fig. 2, and advantageously as an improvement upon and using the "process for preparing a concentrated fertilizer" described in U. S. Patent No. 1,194,077 dated Aug. 8, 1916, duly dedicated to the public, without cost, by the inventors W. H. Ross, and A. R. Merz and J. N. Carothers, of the U. S. Department of Agriculture. Quoting from said patent:

"A concentrated fertilizer is thus obtained 35 directly in the dry way without the aid of scrubbing towers of any kind, and all expenses involved in the evaporation of solutions, filtration and the drying of crystallized salts, operations which are incident to the 40 preparation of salts by the wet method, are avoided. \* \* \* When the process is carried out under suitable conditions, the solid product resulting from the reacting gases (i. e.,  $P_2O_5$  plus  $2NH_3$  plus  $H_2O$  or  $2H_2O$  or 45  $3H_2O$ ) settles out in a very flocculent condition, which enables it to be easily collected \* \* \* by filtering the gases with the suspended solids through a porous medium, or by an arrangement of baffle plates. \* \* \*

50 We do not confine our process to the production of ammonium metaphosphate or to any other definite compound of phosphorus oxide and ammonia, for there may be produced in the dry state, any one of several compounds, 55 or a mixture, of different compounds by causing variations in the relative amounts of the reacting gases."

When it is desired to retain most of the phosphates in the slags, to be utilized as slag 60 phosphate fertilizers, I add basic materials to the mixture, especially such as have a fertilizer value, such as lime or calcite or magnesia or the like, in calculated amount, advantageously so that the total of the basic 65 elements shall be approximately double the

acid elements, silica and the like, and plus the amount of phosphoric acid content, to be fixed by the lime or magnesia or the like.

On the other hand, where it is desired to volatilize the phosphoric acid, I provide excess of the acid constituents, sufficient to combine with the basic lime and the like, and recover the phosphoric acid values as described for Fig. 2; advantageously combining the vapors with gaseous ammonia, 70 upon the due cooling of the vapors, and duly forming a phosphate of ammonia, a most concentrated fertilizer; the said vapor  $P_2O_5$  is negatively charged by the emission of positive electrons due to heat of slags; 80 and thereafter upon bringing such in contact with the  $NH_3$  gases, either electrically neutral or negatively electrified, in the insulated recovery apparatus, and mixing conduits described, and advantageously as de- 85 scribed in above Patent No. 1,194,077 the desired compound is attained, with molecules of increased density and stability. Such vapors may also be recovered in water, in well known methods; and advantageously 90 injecting steam into the vapors in an insulated conduit as described. As a general rule, like the above  $P_2O_5$  molecules which emit positive electrons at high heat, and become negatively charged, so also in general 95 do  $SiO_4$  in silicates, and  $CO_3$  in carbonates, and  $SO_4$  in sulfates, and uncombined Fe, and Cl, and Fl, and  $NO_3$ , and CN; and on the contrary, like CaO which emits nega- 100 tive electrons at high heat, so also in general do Fe in ferrous or ferric compounds, and Mn in manganic compound H and K, and Mg, and Na, and  $NH_4$ , and  $K_2O$ .

The process is operated in an analogous manner for the utilization of the heat of 105 molten slags and the hot gases from the source producing the slags, in the recovery of values from potash-bearing siliceous or basic rocks, or the like; though advantageously at lower temperatures.

Quoting from Bulletin No. 415, U. S. Department of Agriculture 1916, on "The recovery of potash from alunite."

"Alunite is a hydrous sulfate of potash and alumina. On heating to a moderate 115 temperature (500 C.), water is driven off and the mineral decomposes into alumina and potassium aluminum sulfate. Upon increasing the temperature to 700 to 750 C., the latter compound is decomposed, fumes 120 of sulfur dioxide and trioxide are evolved, and a residue remains which consists of alumina and soluble potassium sulfate, \* \* \* and the residues subsequently 125 leached with water. A temperature between 750 and 800 C. was found to be best for the complete extraction of the potash with the minimum amount of water."

In the application of my electrical process to molten slags and alunite, I follow the 130

- general process heretofore described, empirically first advantageously mixing equal weights of each; and at low temperatures 700° to 800° C., where open top slag mixing 5 vessels only are available; and either using the mixture, upon due granulating or pulverizing, as a fertilizer, without effecting a separation of the soluble potash salts; or I may duly leach the latter therefrom.
- 10 Where apparatus such as Figs. 2 or 3, is available, for collecting and recovering values from emanations, I advantageously, treat the mixtures at the higher slag temperatures 1000° C. upward, with excess of 15 bases, and minimum of acids, silica and the like, to vaporize the alkalis with other emanations, and recover the values as described.

It will be noted, that in the process, I advantageously first utilize the heat to duly calcine such rocks or the like, to first drive off the water and the oxids of sulfur, or the like by volatilization, at the start, prior to the due recovery of values. The residue, 25 after the complete volatilization, is suitable for making metallic aluminum.

Quoting further from said U. S. Bulletin 415:

"Potash is now being recovered as a by-product from blast-furnace operations and in the manufacture of cement from potash-bearing silicates, lime being used to convert the potash into oxid, in which form it is readily driven off. The residue then consists of a clinker having the properties of hydraulic cement."

In the application of my electrical process to such, I advantageously blow such with the waste gases from the furnace or the like through the molten mixtures as described; or where gathered in the form of dusts at their source, I duly mix same, as described for other materials, with the addition of lime or other base, where such is indicated.

Quoting further from said U. S. Bulletin 415:

"Alunite and fluorspar or some other fluorid are powdered and intimately mixed, 50 (or better, are ground together) and heated at such a temperature that the hydrofluoric acid (of the fluorid) is set free by the sulfuric acid (or sulfur trioxid) yielded by the alunite on heating. \* \* \* This converts 55 the alumina into aluminum fluorid the potassium remaining as sulfate. The product is then leached, the potassium dissolving as sulfate."

This latter utilization of fluorspar, is the 60 invention of Paul J. Fox of the Department of Agriculture, duly dedicated to the public, as described in U. S. Letters Patent No. 1,217,432, dated February 27, 1917; and the use of fluorspar or the like is utilized in my

process, where the economic conditions are 65 such, that the spar can be economically transported to the source of the molten slags, in order to there utilize the heat and heat-emitted electrical conditions of this invention, and in order to economically recover the values desired from alunite and from other materials herein indicated. And in order that such heat effects may be utilized at the molten slag sources, I advantageously utilize the materials from which 70 values are desired to be recovered, with such additive fluxes or the like admixtures, 75 economically attainable in different and distant sections of the country,—and which materials as well as fluxes must be different on 80 account of costs of transportation. In the U. S., alunite is often associated with gold ores. I also mix fluorspar with phosphorites and slags, for like reasons. Or spar and calcite.

Said Bulletin 415 gives the analyses of sundry alunites, with potash (K<sub>2</sub>O) content varying from 3.48 to 9.61%; and silica 39.20 to 4.41%; and iron and aluminum oxids 26.97 to 36.10%; water about 13%.

Other materials with potash content, available in some sections, are sericite or potash slates. An analyses of such and of the available molten slags, will readily enable the operator to determine the amounts 95 to mix, and of desirable fluxes. In the application of my process, I advantageously mix the slags with about one-half the weight of the slates; and add lime thereto in amount about three and a half times the 100 amount of lime or magnesia in the slags and slates combined, and after first mixing and fusing such then add common salt in amount one half said added lime; and preferably at over 1310° C. in order to fuse the mixture; after the fusion, I advantageously reduce the temperature to about 800° C. and stir and agitate for about 20 minutes, advantageously recovering values from the vaporizations of potassium chlorid 110 fumes; and also sodium chlorids; and quickly cooling and granulating the residues, from which potassium chlorids can also be duly leached and crystallized 115 out upon due evaporation. Or by dispensing with the salt, and quickly cooling and granulating the mixture after the fusion, the potash may be obtained in soil soluble state to amount of about 10 to 12% or more, of the granulated or pulverized 120 mixture, suitable as fertilizer. In the first mixture with the potash material, I adjust the unipolar earthing device to carry to earth the heat emitted negative electrons, leaving the potash molecule positively 125 charged; and when such meet the neutral or negative chlorine (and which latter is readily charged negative, emitting positive elec-

trons at high heat,) then the compound potassium chlorid is attained, and with increased density and stability.

Where the potash bearing "leucite" rocks 5 are economically available for compounding with molten slags, I apply my process to the compounding thereof, substantially as above described *i. e.*, after fusing coarsely ground rock advantageously with double its weight 10 of molten slag and adding lime or the like base in double the amount of calculated lime or lime and magnesia in the combined slags and rock, and so doing at the highest slag temperature, and with the unipolar earth- 15 ing device adjusted to earth negative electrons; then and advantageously at lower temperature, add common salt in amount about one third the weight of the added lime,—the latter being advantageously added 20 without any earth connection, from the mixture; *i. e.*, by opening ground switch of the unipolar earthing device, or otherwise disconnecting same from the mixing chamber.

Leucite is a potassium alumino-silicate, 25 usually found in lava flows.

Where the potash bearing "green sands" are commercially available, I mix and treat same as above indicated; and advantageously mix such, (as also any other potassium bearing silicate rocks), as recited in 30 Fig. 2 apparatus, in one separate molten slag chamber,  $S^2$ , and with suitable admixtures of fluxes lime or the like, and in another slag mixer  $S^1$ , likewise mix a phosphorite material as above described; and thereafter, duly mix the two in a third chamber  $S^3$ ; and simultaneously, collect and treat the combined emanations from the three mixing chambers; and recover the 40 values from each; including potassium phosphates, from the third chamber residues, and the emanations therefrom.

Quoting from Technical paper No. 187 of 1918, of the U. S. Bureau of Mines, entitled "Slag viscosity tables for blast furnace work:"

"The most important conclusion to be drawn from the results of the investigation, is, that a slag, even when melted and completely converted into a liquid, is composed of relatively complex compounds of lime, alumina and silica, and not of a simple mixture or solution of the constituent oxids of  $CaO$ ,  $Al_2O_3$  and  $SiO_2$ . \* \* \* this discovery will ultimately necessitate a revision of ideas commonly held regarding the chemical properties of slags, etc."

I avail myself of said discovery, by advantageously adding admixtures to the mixtures of molten slags and materials comprising values to be recovered, by the addition of other materials in the nature of fluxes as described to insure compounding

of the values with the latter and to attain 65 chemical reaction and other compounds

with the latter, together with electrical adsorption compounds of the values with the complex compounds of lime, alumina and silica, above indicated, and with the minute crystalline particles of such or of the admixtures, which may not be completely fused 70 at the lower molten slag temperatures.

Quoting further from said paper No. 187:

"Within the temperature range, beginning at a point where the ternary eutectic 75 melts, and extending to a point where the entire mass is converted to a liquid, we are dealing with a complex system, (*i. e.*, molten slags), composed of a liquid within which is suspended a certain quantity of 80 solid crystals, or if the amount of the eutectic is small, of a mass of crystals covered on the surface with a thin layer of liquid slag."

Again quoting from said No. 187:

"It is known that the calcined limestone 85 of the charge, the gangue of the ore, and the ash of the coke, are fused into a viscous mass, known as slag, \* \* \*.

"The molten iron globules, entrapped within the highly heated slag, are thereby raised 90 to a temperature considerably above the melting point of pig iron. During the time the molten iron is in contact with the slag within the blast furnace, those reactions of desulfurization and of silica reduction occur, 95 that determine the grade of pig produced."

I advantageously facilitate the said reactions and the like with the application of my above described process and apparatus 100 applied to such furnaces and smelters  $Z$  and the like, as shown in Fig. 2.

I do not restrict the process to hot molten slags, from iron furnaces, steel converters, or the like, but also utilize such from copper 105 smelters or converters, whose slags consist mainly of silica, lime and ferrous oxid, with minor quantities of alumina and other oxids: and also slags from lead smelters, and other metallurgical operations. And likewise as 110 regards the emanations, vaporizations hot gases or the like, from such furnaces or the like, sources of molten slags, the high heat whereof, and the heat-emitted electrons and ensuing electrifications are utilized, similarly, as described, and as illustrated by the apparatus of Fig. 2; and advantageously, by blowing such emanations and hot gases, from the smelter stacks or the like, under insulated 115 conditions, advantageously first electrified 120 with one sign only, and then projected through the molten slag mixtures, through suitable insulated twyers, and advantageously before utilizing the hot waste gases for heating steam boilers, or for preheating 125 blasts, or preheating or warming the materials to be mixed with the slags; or other uses.

Gases which have been in contact with glowing slags, either in the smelter or con- 130

verter or other source, are ionized thereby, and become conductors; I avail myself thereof in the manner above described; and to neutralize heat-emitted electrons in the slag mixtures, and subsequently, in the emanations carried into the recovery apparatus by the blasts of gases, as illustrated in Fig. 2; and which may be similarly used with retort-like vessels such as Fig. 3 and in the conduits of the recovery apparatus, I earth from such emanations and gases, electrons of one sign only, by bringing same in contact with the unipolar contact and earthing device, and with ensuing desired compoundings with other neutral or oppositely charged gases or the like. The denser the gas, the greater the number of electrons, and the greater the number of collisions and ensuing electrical compounding and which are advantageously increased by suitable regulable blower pressure, in the conduits, with resulting increased density and stability of the molecular products.

I conduct the process as regards the electrified gases, in sundry ways, depending upon the values to be recovered. Thus, the hot gases and accompanying emanations from the smelter "Z," in Fig. 2, or like source of molten slags, from contact with the latter, comprise heat emitted electrons of both signs in general, and at a temperature exceeding 750° C.; and I advantageously first earth therefrom, in a suitable conductor gas conduit section P<sup>4</sup> details not shown, preceding the twyer T<sup>1</sup> leading to slag mixture S<sup>1</sup>, with phosphorites, the negative electrons; and similarly another stream of the hot gases is projected into slag mixture S<sup>2</sup>, with potash or the like, through twyer T<sup>2</sup>, preceded by a conductor gas conduit section P<sup>5</sup>, details not shown, having a unipolar earthing device to earth positive electrons only; thereupon the electrified gases take up from the mixture while being projected therethrough, the heat emitted electrons of opposite sign, neutralizing many such, and carrying off the surplus if any not neutralized; and generally the latter, as there is a great excess of electrons from the molten solids as compared to gases.

As the gases are projected through S<sup>1</sup>, and S<sup>2</sup>, into emanations and gas conduits G<sup>1</sup> and G<sup>2</sup> respectively, and then into the common mixing conduit or other gas mixing device G M, the opposite electrons are again earthed from G<sup>1</sup> and G<sup>2</sup>, or conduit sections P<sup>6</sup> and P<sup>7</sup> thereof respectively so that when the gases are mixed in G M, which is neutral or completely insulated, they are oppositely electrified, and compoundings are readily and quickly effected, with molecules of increased density, resulting in increased stability; and thereupon and thereafter values are recovered more quickly and effectively, in increased amount. The said gas conduit sec-

tions are advantageously provided with insulator dielectric joints D J at the ends, with due connection with ensuing pipes or vessels; and advantageously regulable valves in the dielectric joints, not shown, to duly enlarge 70 or diminish or cut off the flow of the gases; and with insulator supports; and duly electrically connected with E E, a unipolar earthing device, adjustable to earth either plus or minus electrons only, or neither, i. e., 75 with no ground connection.

Again, I may utilize the hot furnace gases, duly electrified by the earthing of heat emitted electrons of one sign only, as described, by the due projection thereof, under 80 suitable pressure, and under insulated conditions, into retort-like chambers with suitable materials or mixtures therein, as in Fig. 3, through inlet conduit "I," and advantageously so doing after, in some cases, duly 85 purifying the gases, as by the prior removal of fumes and dusts therefrom; such blasts of gases thereby serving the function of agitating, as also electrifying by contact or of compounding at high temperatures with emanations from said materials in the retort, and in the ensuing gas mixing coils or the like, and recovery apparatus connected with G<sup>8</sup>, Fig. 3, not shown in Fig. 3, but substantially 90 as shown and explained for and in Fig. 2. 95 And further, in some cases, I inject, as through injectors G J Fig. 2, and Fig. 3, streams of other gases or vapors, etc., either neutral or oppositely electrified, and under insulated conditions (and previously duly 100 heated by means not shown of hot waste gases or the slag heats), into contact with the first electrified hot gases, or emanations from mixtures, for due electrical compounding therewith, and the recovery of values 105 therefrom as previously described. Thus where the materials treated as described comprise sulfid ores or rocks, which when highly heated or fused, emit sulfur gases in sufficient amount to be economically of value, 110 treat the gases and emanations as described, advantageously by earthing heat emitted negative electrons therefrom and recover same duly, as sulfuric acid by the compounding with water vapors advantageously neutral; or by compounding with ammonia gas, 115 where such is economically available, to make ammonium sulfates, for fertilizer use. In said cases, I advantageously apply my electrical method as described, to and in the 120 "Process for the manufacture of sulfuric acid," invented by William H. Wagaman, of the U. S. Department of Agriculture, described in his U. S. Patent 1,185,029 dated May 30, /16, and duly dedicated to the public. 125

The sulfur gases are advantageously electrified positive, by the earthing of heat-emitted negative electrons, as described above; and are brought into contact with, and mixed with steam vapors, advanta- 130

geously neutral, and thereafter absorbed in water to make sulfuric acid. And likewise, the positively electrified sulfur gases and emanations are brought into contact with 5 negatively electrified ammonia gases; and including ammonia or the like gases in the blast furnace gases blown through the molten slag mixtures comprising sulfur compounds, making a crude sulfate of ammonium fertilizer, or the like.

It will be understood, that electrification of components of compounds, herein indicated, is attained in some cases by the due earthing of the heat emitted electrons, and 10 advantageously the negative; and again such heat-emitted electrons from one molecule or element or atom, may be neutralized by the opposite from a neighboring particle; or such may be projected into, or taken up by a 15 neighboring atom or molecule or particle coming into contact therewith, and thereby charging or electrifying the latter, advantageously positive, *i. e.*, when it takes up a positive electron while neutral, or on the contrary negatively charged when it, being neutral, takes up a negative heat-emitted electron. In the case of slag mixtures, and others herein described, it is advantageous 20 to determine such empirically, and conducting the process, by following at the start, the general rule, that the heat emitted electrons are negative from or of the bases or basic oxids,  $\text{CaO}$ ,  $\text{MgO}$ ,  $\text{Na}_2\text{O}$ ,  $\text{K}_2\text{O}$ , or the like or basic radicals; also from  $\text{NH}_4$ ; and 25 that in general, the heat emitted electrons are positive from the acid oxids or acid radicals; such as  $\text{P}_2\text{O}_5$  and the oxids of C, of Si, of S, and some of the oxids of N, and  $\text{NO}_2$  and  $\text{N}_2\text{O}_5$ , and some of the oxids of manganese, and of chromium; and of some elements as  $\text{Cl}$ ,  $\text{Fl}$ , and others.

It has been noted that the ionizing power or effect of the positive electrons, emitted by the high heat, upon the neighboring or 45 contacting gases or other medium into which such are emitted, is far greater than the negative emissions, sometimes in the ratio of 100 to 1. I avail myself of this property, as illustrated in the process with 50 phosphorite mixtures, whereof the phosphates emit positive electrons, especially the vapors, and which facilitates ensuing recoveries; and likewise with plain iron Fe which in the smelter emits mostly positive 55 electrons, some of which are emitted into the escaping gases and emanations, duly utilized as described; and again where comparatively cold gases or vapors, are to be combined with the hot gases in the conduits 60 of recovery apparatus, and such are advantageously to be ionized, I advantageously bring such in contact with an iron conduit at glowing temperature to attain emission of positive electrons therefrom into such, 65 prior to the compounding.

And further, where it may be optional, as to which electron to earth, where both are emitted, and especially where a compounding is to be effected with a neutral substance, then I advantageously earth the negative 70 emission in the manner described, so as to leave the more powerful positive electron to perform the desired function, in electrically facilitating the formation of the desired compound or product, in the manner 75 described. Where two gases are thus compounded, either one being ionized, or each electrified with opposite signs, the compounding is facilitated by the injection into the gases of steam or sprays of water or 80 other desirable liquid disperse medium or solvent, as the drops of water or the like, facilitate the condensation of the ions of the gases thereon together with simultaneous or ensuing compoundings. It is well 85 known that the chemical combination of gases is enhanced by the presence of moisture; I avail myself of this property, in combination with the electrifications advantageously attained as described, by the due 90 earthing of heat-emitted electrons of one sign only, and conducting the compoundings under insulated conditions, as described.

I am aware of "the utilization of acid and 95 basic slags in the manufacture of fertilizers," such being also the title of Bulletin No. 93, Bureau of Soils, U. S. Department of Agriculture, by Wm. H. Wagaman, of 1913; and I do not claim any such slag-fertilizers, excepting when made under my 100 electric process herein described, and the improved fertilizer products electrically fixed, of increased density and stability, and of diminished hygroscopicity, as compared to the same made or attempted or recommended to be made without such process but as heretofore. Moreover, the commercial basic slags heretofore used as fertilizers are such as obtain their phosphate content 110 from the ores in the smelting thereof or the like, and not by subsequent mixings.

I claim—

1. The process of electrically utilizing hot 115 limpid molten slags in the compounding thereof with other materials comprising values to be recovered, which consists in suitably mixing and largely fusing the materials, in and with the slags; and simultaneously, during the mixing, electrically 120 carrying to earth, or otherwise neutralize, the heat emitted electrons of one sign only; all under insulated conditions; and thereafter recovering the values from the mixture and from the emanations, the fumes, 125 vapors, dust, gases or the like.

2. The process of treating and utilizing molten slags, which consists in mixing and compounding the slags with suitable materials comprising values, and so doing 130

under electrically insulated conditions; and thereafter suitably recovering values from the mixture and emanations therefrom.

3. The process of treating and utilizing 5 molten slags, which consists in mixing and largely fusing in the slags, other materials having values and previously warmed; and so doing under electrically insulated conditions; and thereafter suitably cooling, 10 granulating, pulverizing or otherwise preparing and utilizing the mixture.

4. The process of electrically utilizing a molten slag, in the compounding thereof with other materials, which consists in 15 largely electrifying the slags through duly grounding therefrom, heat emitted electrons of one sign only, prior to the compounding; and thereafter duly mixing the slags with other materials having values to be recovered; and with the admixture of suitable 20 fluxes for the latter; and so doing under insulated conditions; and thereafter, duly recovering the values from the mixture and the emanations.

25 5. The process of treating and utilizing molten slags, which consists in mixing the molten slags with other materials comprising values, and with gases, and so doing under electrically insulated conditions; and 30 thereafter suitably recovering values from the mixture and separately from the emanations therefrom.

6. The process of electrically utilizing 35 molten slags in the compounding thereof with other materials comprising values, which consists in electrifying material portions of the slags prior to the compounding, through earthing therefrom a large part of the heat-emitted electrons of one sign only; 40 and simultaneously repulsing and retaining the opposite sign; and thereafter mixing the slags with other materials comprising values; and thereafter, and during such mixing, agitate the mixture with streams of 45 gases blown therethrough; all under insulated conditions; and thereafter recovering values from the mixture and from the emanations therefrom.

7. The process of electrically utilizing 50 molten slags, which consists in mixing the molten slags with other materials comprising values, and with hot gases, all under insulated conditions, the slags having been previously largely electrified with one sign 55 only, and the gases largely ionized and electrified with opposite sign, by the due earthing of heat-emitted electrons from the slags and simultaneously repulsing and retaining electrons of opposite sign, and separately 60 from the gases, prior to the mixing; and thereafter, separately duly recovering values from the mixture and from the emanations therefrom, under insulated conditions.

65 8. The process of electrically utilizing

molten slags, while hot and limpid from its smelter or converter or like source, which consists in mixing the slags with other materials comprising values and with suitable fluxes for the latter, and agitating the mixture with streams of hot gases from the same source; and so doing under insulated conditions; and thereafter suitably recovering values from the mixture and separately from the emanations therefrom. 75

9. The process of electrically utilizing molten slags, which consists in the convection of heat and its electron emitting effects, to suitable materials or mixtures of materials, comprising values, through an intervening conductor solid plate or retort or other container holding the materials and the said solid only being in direct contact with the slags, and after the solid plate container and the materials have been thereby 80 raised to a sufficiently high temperature to cause the emission of electrons therefrom and while agitating the materials, then duly earth such electrons of one sign only from the materials, and simultaneously agitate the 85 materials; all under insulated conditions and thereafter recovering values from the materials and emanations therefrom.

10. The process of treating and utilizing the heat of molten slags, in the recovery of 95 values from suitable materials, including mixtures of materials and suitable fluxes therefor, which consists in subjecting the materials, contained in a suitable vessel of conductor substance, to a bath in the molten 100 slags without direct contact, with the latter, of the materials; and after the conductor vessel has thereby been raised to a high temperature, then pass therethrough, and simultaneously agitate thereby, sundry hot waste 105 gases from the furnace source of the slags, and which gases have been previously ionized and electrified, with one sign only; all under electrically insulated conditions; and thereafter recover values from the materials 110 and from the emanations therefrom.

11. The process of electrically utilizing a molten slag, which consists in bringing gases into contact therewith, by blowing gases therethrough, under insulated conditions, 115 and thereby ionizing the gases, and simultaneously and thereafter earthing therefrom, heat-emitted electrons of one sign only, and thereafter recovering values from the gases under insulated conditions. 120

12. The process of electrically utilizing molten slags, which consists in bringing gases into contact therewith and thereby ionizing the gases, and simultaneously and thereafter earthing from the gases and accompanying emanations from the slags and gases, the heat emitted electrons of one sign only; and thereafter mixing and compounding such with other gases which have been similarly brought into contact with another 125 130

batch of molten slags, and whose heat emitted electrons of opposite sign to the above have been previously duly earthed during and after such latter contacts; and therefore 5 after duly recovering the values from the mixture of the gases; and all under insulated conditions.

13. The process of electrically utilizing molten slags, which consists in bringing the 10 hot waste gases from the smelter or other source of molten slags, with their heat-emitted electrons, into contact with a unipolar contacting and earthing device, in and from a suitable conductor conduit and to 15 earth therefrom electrons of one sign only; and thereafter recovering values therefrom and therewith; and all under insulated conditions.

14. The process of electrically utilizing 20 molten slags, which consists in bringing hot gases and accompanying emanations from the insulated converter or other source of molten slags or of highly heated gases, and with their heat emitted electrons due to 25 said source, into contact with a unipolar contacting and earthing device, to earth from the gases, electrons of one sign only; and simultaneously repulse and retain opposite electrons; and thereafter projecting 30 the gases and accompanying emanations thus previously electrified with one sign only, into and through contact with other agitated suitable materials including gases or emanations, or the like, comprising values 35 or mixtures of such materials; and all under insulated conditions; and thereafter recovering values from all such, including the compounds thereby formed.

15. The process of treating and utilizing 40 molten slags in the compounding thereof with suitable minerals comprising fertilizer ingredients, which consists in mixing the molten slags with the minerals and suitable fluxes therefor, all previously pulverized 45 and warmed, and agitating the mixture until the minerals have been largely fused; and so doing under electrically insulated conditions; and thereafter, duly granulating and pulverizing same for fertilizing use.

50 16. The process of electrically utilizing hot limpid molten slags in the compounding thereof with suitable minerals comprising phosphatic ingredients or values, capable of being made available as fertilizers, which 55 consists in electrifying the slags negatively, by suitably earthing therefrom heat-emitted electrons of opposite sign, and thereafter mixing such slags with the minerals and suitable fluxes therefor, duly ground and 60 warmed, and agitating the mixture to insure heat emissions of electrons from the minerals during the mixing and fusion thereof; and so doing all under insulated conditions; and thereafter duly granulating 65 the slag mixture.

17. The process of electrically utilizing molten slags in the compounding thereof with suitable siliceous or basic minerals comprising phosphatic values, which consists, in first duly earthing from the molten 70 slags, a large portion of the heat-emitted electrons of one sign only, and thereafter mixing such slags with the minerals, previously duly comminuted and warmed, and duly agitating the mixture thereby attaining 75 homogeneous heat, and agitating until heat-emission of electrons ensue from the minerals and the fusion thereof; and so doing all under insulated conditions; and thereafter duly granulating the mixture 80 and treating the grains while suspended in streams of hot gases and emanations from a like mixture; the latter step under insulated conditions, and then plunged by gravity into cold water. 85

18. The process of electrically utilizing molten slags in the compounding thereof with suitable minerals comprising potash values, which consists in first duly earthing from the molten slags, a large portion of the 90 heat-emitted electrons of one sign only; and then duly mixing such slags at suitable temperature, with the minerals and suitable fluxes therefor, all previously ground and warmed; and duly agitate the mixture a 95 material time to attain homogeneity of heat, and near-fusion, and heat-emitted electrons, and emanations including some potash volatilizations; all under insulated conditions; and thereafter suitably recover the values 100 from the emanations under insulated conditions; and separately utilize the values in the remaining slag-potash-mixture while still molten, by duly leading to earth therefrom and upon further agitation, the heat-emitted negative electrons, and thereafter duly mix the same with a like slag-phosphate mixture while molten, and from which the heat-emitted positive electrons have been 105 duly earthed prior to the mixing of the two batches; and the mixing being conducted under insulated conditions; and thereafter duly granulating the mixture of the two batches. 110

19. The process of electrically utilizing 115 molten slags in the compounding thereof with suitable minerals comprising phosphatic values, and with other minerals comprising potash values, which consists in first making separate batches of molten slag mixtures of the phosphate minerals and separately of the potash minerals at a lower temperature; and during the mixing of each batch, duly earth from the potash mixture, the heat-emitted negative electrons, and duly 120 earth from the phosphate mixture, the heat-emitted positive electrons; and thereafter, duly mix the two batches of molten slag mixtures; and all under insulated conditions; and thereafter duly granulate the 125 130

mixture of the two batches and further separately collect the emanations from each batch and from the mixture of the two batches, and intermix all emanations under 5 insulated conditions; and duly recover the values therefrom.

20. In the process of electrically utilizing molten slags in the compounding thereof with other materials comprising values to be recovered, the steps of agitating the molten slags and simultaneously earthing therefrom heat-emitted electrons of one sign only, and thereafter causing the molten slags to flow and overflow in thin wide streams in a suitable 10 space, and simultaneously injecting blasts of materials, previously warmed and comminuted, into the falling streams of molten slags; and all under insulated conditions.

21. In the process of electrically utilizing 20 molten slags in the compounding thereof with other materials comprising values to be recovered, the step of treating the emanations from the hot molten mixture under insulated conditions, and of duly driving the 25 emanations against baffle wires or sieves or plates or the like in the path of the moving emanations, and simultaneously earthing from the baffles, electrons of one sign only, being the same sign as that of the prevailing 30 heat-emitted electrons in the emanations; and finally after the due precipitations of dusts and flocculations or the like from the moving emanations, duly driving the remaining gases of the emanations after 35 duly recovering values therefrom, against and into contact with coarsely comminuted or granular masses of solid adsorbents of one sign, followed by like passage and contact with comminuted solid adsorbents of the 40 opposite sign; all under insulated conditions.

22. In an apparatus for electrically utilizing molten slags in the compounding thereof with other materials comprising values to be recovered, a slag mixing chamber 45 of a suitable vessel, on insulator supports, with a conductor refractory lining of the chamber, with means of feeding molten slags into the chamber and of withdrawing molten mixtures therefrom; with 50 means of feeding and supplying other materials in comminuted form into the molten slags in said chamber; with means of agitating the molten slags and the mixtures in said chamber; with means of electrically 55 earthing from said slags and from said slag mixtures and from any mechanical agitator and the conductor lining in contact with the slags, the heat-emitted electrons of one sign only; and simultaneously repulsing and 60 retaining opposite electrons; with means of blowing hot gases through twyers into the molten mixtures; with means of collecting and leading away and duly treating and recovering values from the heat-emanations

from the slag mixtures; with insulator supports for all connecting apparatus; with dielectric joints in connecting piping to attain operating under insulated conditions, with means of granulating, and cooling the slag mixture residues, and of suitably recovering 70 ing desired values therefrom.

23. In an apparatus of the nature described, a slag mixing unit of the character described, with electric means of earthing from mixtures of one kind, in its chamber, 75 the heat emitted electrons of one sign only, in combination with another slag mixing unit holding a different slag mixture, with means of earthing from the latter, heat emitted electrons of opposite sign; with further 80 means of duly mixing in a similar slag mixing unit, under insulated conditions, without earthing connection, the two aforesaid molten slag mixtures; with suitable means for the recovery of values from the final 85 mixture, and separately from the emanations therefrom; with means of combining the emanations from each of said units, and of recovering the values therefrom.

24. In an apparatus of the nature described, a molten-slag pot, or the like, with open top, with insulator supports, with a conductor refractory lining of the chamber of pot, with a suitable mechanical rabble with insulator handle, the rabble and the 95 pot shell being of metal of higher melting point than the slags and with means of electrically connecting the rabble and the shell and conductor lining with one pole of a direct current circuit whose other pole is 100 earthed.

25. In an apparatus of the nature described, a slag run for conveying molten slags from source thereof to a slag mixing chamber, comprising an open conduit, with 105 insulator supports with conductor refractory lining, with conductor baffles in the run-way contacting with the flowing slags and with means of electrically connecting the baffles and conductor lining and the metal parts 110 of the conduit, with one pole of a direct current circuit, whose other pole is earthed.

26. In an apparatus of the nature described, a flue for the emanations, including hot fumes dust gases or the like and from 115 molten slag mixtures, in combination with insulator supports, with a conductor refractory lining of flue, with dielectric joints for connecting apparatus, with suitable metal baffles including wires suspended from insulator supports in the flue passage ways for the emanations, together with the metal shell or frame of the flue and its conductor refractory lining electrically connected with one pole of a direct current circuit, the other pole being earthed; with means of removing 120 from the flue, the fumes, dust, flocculations or the like precipitated therein.

27. In an apparatus of the nature described, in the flue to chimney for the emanations from molten slag mixtures after the fumes dust flocculations or the like have 5 been removed, two consecutive U shaped conduit joints, with dielectric joints therebetween, and also at the terminals connecting with the flue, with conductor refractory lining of conduits with insulator supports 10 for the conduit joints with coarse comminuted granulated solid adsorbents of conductor substances in the bends of the U of the conduits, with means of electrically connecting the adsorbents and the metal frame 15 of the conduit joints and the conductor lining thereof with one pole of a D. C. circuit, whose other pole is earthed, and the earthed pole of the one circuit being opposite in sign to the other circuit's earthed 20 pole, with means of accelerating the passage of the waste gases through the passageways of the adsorbents and into the chimney; with means of cooling the said conduit joints, and of collecting therefrom any 25 depositions, and of replacing the said adsorbents therein.

28. In an apparatus of the nature described, a conduit pipe for conveying hot waste emanations, fumes, dust, gases or the 30 like from a smelter or converter or furnace or the like, to a slag mixing chamber, with a conductor refractory lining of the pipe, with means of blowing the emanations through suitable twyers into the slag mixtures, with means of earthing from the said emanations while passing through said conduit, heat-emitted electrons of one sign 35 only; with insulator supports for said conduit; with dielectric joints at the terminals 40 connecting with the twyers.

29. In an apparatus as described, means of withdrawing from a molten slag mixing chamber, mattes and metals of greater specific gravity than the slags, and which settle by gravity to the bottom of said chamber; and which means comprise a suitable 45 exit pipe from the bottom of the chamber, with cut-off valve, with a suitable receiving receptacle for molten mattes and metals; in combination with a slag mixing unit, and means of earthing therefrom from the agitator rabble and conductor lining the greater part of the electrifications of particles due to the heat thereof and prior treatment.

55. 30. In an apparatus as described, means of collecting the emanations from molten slag mixtures and of recovering the values from the emanations, in combination with insulator supports of all apparatus and conductor linings of conduits and flues which contact with the emanations in the collection and recovery processes, while still hot, and with means of earthing heat emitted electrons of one sign only from any part of 60 the apparatus during the treatment.

31. In an apparatus as described, an injector with insulator supports for projecting sand-like particles of materials into molten slags while passing and falling into suitable chambers over suitable guiding 70 plates, the latter being electrically connected with means of electrically earthing therefrom and from the slags in contact therewith, heat-emitted electrons of one sign; with means of connecting the injector with 75 a unipolar earthing device, to earth electrons of opposite sign only.

32. In an apparatus as described, a retort-like vessel of conductor metal of higher melting point than slags, with insulator supports, with conductor refractory lining of the vessel, with means of setting such in a bath of molten slags, in and with a slag-pot on insulator supports and lined with refractory substances, means of replacing and 80 attemperating the molten slags, means of introducing into the chamber of the retort suitable materials or mixtures of materials having values to be recovered; means of stirring and agitating the mixture of materials in the retort; means of blowing hot gases into and through and comminuted materials into the retort; means of withdrawing materials from the retort; means of 85 electrically connecting the materials 90 within the retort and the conductor refractory lining, during the mixing and agitation and fusion thereof, to earth therefrom heat-emitted electrons of one sign only; means of collecting the emanations from the 95 heated and fused materials through the neck of the retort into suitable apparatus for the recovery of values from the emanations; means of withdrawing the remaining material from the chamber of the retort, and 100 means of recovering values therefrom.

33. In an apparatus for the purpose described, an open-top kettle-like vessel, made of a substance having higher fusing point than slags, with a conductor refractory lining, with means of setting such in a bath of molten slags held in a slag-pot with insulator supports, a water-cooled mechanical stirrer for stirring materials in the kettle, and means of blowing hot gases through the 110 stirrer, the stirrer being made of conductor metal of higher melting point than slags, means of electrically connecting the conductor lining and the stirrer with a unipolar earthing device to earth heat-emitted electrons of one sign only; means of attemperating the contents of the kettle, and of the slag bath, cooling coils or the like suitable for utilizing waste heat for generating steam.

34. In an apparatus for the purpose described, a metallurgical slag-producing furnace, with insulator supports including insulated means of feeding charges thereto, including blasts of gases, or hot air, and for withdrawing slags therefrom; means of con- 125 130

vveying the slags, from the slag-tap of the furnace, into a detached slag-run trough on insulator supports or the like, means of electrically connecting the molten slags in said 5 furnace and in said trough with a unipolar contact and earthing device to earth therefrom heat-emitted electrons of one sign only.

35. In an apparatus for the purpose described, a suitable container for molten slags 10 and molten slag mixtures, on insulator supports with conductor refractory lining, in combination with means for bringing the molten slags in contact through said lining with a unipolar contacting and earthing device, adjustable to earth therefrom, heat-emitted electrons of one sign only, and to simultaneously repulse electrons and electrified particles of opposite sign.

36. In an apparatus for the purpose described, a suitable container, including conduits, flues or the like, for treating hot emanations from molten slag mixtures, including from metallurgical furnaces, retorts or the like sources of hot emanations of 25 fumes, dusts, gases and electrons or the like, in combination with insulator supports for the containers and connecting apparatus with conductor refractory linings thereof; with means for bringing the emanations in 30 contact with the conductor lining electrically connected with a unipolar contacting and earthing device to earth from the emanations electrons of one sign only, and simultaneously repulse electrons and contacting particles of opposite sign.

37. In an apparatus for the purpose described, a suitable retort or the like container with conductor refractory lining, set in a bath of molten slag with insulator supports, 40 and holding suitable materials from which values are recoverable by heat and accessory means, in combination with means of injecting ionized gases into the materials, means for contacting the materials through the conductor lining and a suitable stirrer, with a unipolar contacting and earthing device, to earth from the materials, heat-emitted electrons of one sign only, and simultaneously repulse contacting electrons and particles of 45 opposite sign.

38. In an apparatus as described, in combination with insulated conduits or the like for the hot emanations, a suitable injector, with insulator supports, of hot gases, including 55 steam, for projecting such into the emanations while in said conduit, with means of electrically connecting the injector with a unipolar earthing device, to earth therefrom and the gases contacting therewith, electrons 60 of one sign only, and simultaneous repulse of electrons and contacting particles of opposite sign.

39. In an apparatus as described, a molten 65 slag mixing chamber of a suitable vessel, with insulator supports, with a lining of a

conductor material of higher melting point than the molten slags, with means of electrically connecting the lining with a unipolar earthing device, to earth electrons of one sign only, and repulse electrons of opposite 70 sign.

40. In an apparatus as described, a molten slag mixer, comprising a molten slag runway, with slags falling therefrom upon a spreader plate of conductor substance of 75 higher melting point than slags, means of electrically connecting the plate with a unipolar earthing device, means of injecting against the slags while spread upon and falling along the spreader plate, sand-like 80 blasts of materials electrified with sign opposite to prevailing slags and to be mixed with the slags; a suitable slag-mixing vessel to receive the falling mixture; with insulator supports for each part.

41. In an apparatus as described, a mixing conduit for hot gases, with insulator supports, with conductor refractory lining and regulating shut-off valves and dielectric joints at the ends thereof, connecting at one end with 90 an exit conduit leading to suitable recovery apparatus, and at opposite end, connecting with two separate inlet conduits, each of the latter being separately electrically connected with a unipolar earthing device, the one 95 earthing positive electrons only, and the other negative electrons only, and the former with one of the inlet conduits duly joined and connected to lead hot gases and emanations from one mixing chamber wherein the 100 heat-emitted electrons are mostly positive and with the latter one of the inlet conduits duly joined to lead hot gases and emanations from another mixing chamber wherein the 105 heat emitted electrons are mostly negative, the inlet conduits being made of conductor substance of higher melting point than the temperature of the hot gases and emanations, and lined with conductor refractory compound lining.

42. In an apparatus as described, a unipolar contacting and earthing device comprising a direct current circuit, with a pole-changer switch in the circuit to earth one or either pole only; with the other or non-earthing pole electrically connected to a conductor refractory lining of, and to a conductor stirrer in, and to metal parts of suitable vessel chambers and conduits and troughs or the like, on insulator supports, 120 and in combination with and holding agitated hot molten slags and hot gases and emanations therefrom including heat-emitted electrons or the like in contact with said lining or stirrer or the like; with voltmeter, ammeter, galvanometer, resistance, and a manually-operated circuit-breaking switch in the circuit.

43. In an apparatus as described, a unipolar contacting and repulsing and earthing

device, comprising a direct current circuit with means of earthing one pole thereof, and of electrically connecting the other pole with an extensive conductor refractory substance in contact with molten slags or molten slag mixtures or gaseous emanations therefrom, with means of agitation thereof, with insulator supports therefor.

44. In an apparatus as described, a conductor refractory compound lining, comprising principally amorphous carbon uniformly mixed with basic oxids or other fluxes suitable to combine with and promote the fusion of the phosphates and potash or other fertilizer components of molten slag mixtures when contacted therewith upon being treated in the apparatus as described.

45. A mixed fertilizer, finely granulated, comprising a slag, with soil soluble basic phosphate compounds, of chemical combinations and of electrically-adsorbed combinations of phosphoric acid anhydrid gases and basic oxids; and the compounds having increased density and stability and diminished hygroscopicity; and from at least one of the components of which fertilizer there have been removed or earthed prior to or during the compounding, sundry electrons of one sign only.

46. A mixed fertilizer, in granular form, comprising a slag with soil soluble basic phosphate and potash compounds, of increased density and stability, and including electrically adsorbed compounds of anhydrides of phosphoric acid and of potash with particles of slags and of basic oxids; and from at least one of the components of which fertilizer there have been removed or earthed prior to or during the compounding, sundry electrons of one sign only.

47. A mixed fertilizer, in granular form, comprising a slag with soil-soluble basic phosphate and nitrogenous compounds, of increased density and stability and diminished hygroscopicity and increased stability, and including particles with soil-soluble electrically adsorbed gaseous anhydrides of nitrogen compounds; and without ingredients detrimental for fertilizing; and from at least one of the components of which fertilizer there have been removed or earthed prior to or during the compounding, sundry electrons of one sign only.

48. A mixed fertilizer, in granular form, comprising a slag, with soil-soluble basic phosphate, and of potash and of nitrogenous compounds, and including particles with soil-soluble electrically adsorbed gaseous anhydrides of phosphoric acid and of potash and of nitrogenous compounds, and the compounds having high material density and stability, and diminished hygroscopicity; and from at least one of the components of which fertilizer there have been removed or earthed prior to or during the

compounding, sundry electrons of one sign only.

49. An ammonium-phosphate fertilizer compound comprising phosphoric acid gases emanating from molten slag fusions of phosphorite rocks or the like, in electrically compounded combination with ammonia, and the compound including molecules of ammonium phosphate having increased density and stability, and diminished hygroscopicity; and from at least one of the components of which fertilizer there have been removed or earthed prior to or during the compounding, sundry electrons of one sign only.

50. An ammonium-phosphate fertilizer comprising insulated phosphoric acid from which electrons of one sign only have been earthed or otherwise neutralized, prior to the compounding with ammonia, and having increased density and stability, and diminished hygroscopicity.

51. An ammonium-phosphate compound comprising phosphoric acid gases which have emanated from fusions of phosphorite rocks in insulated molten slags, and having heat-emitted electrons of one sign only earthed therefrom, and thereby electrified with opposite sign, prior to due subsequent combination with insulated ammonia previously positively electrified, and the compounded ammonium-phosphates having increased density and stability and diminished hygroscopicity.

52. A mixed granular fertilizer, comprising a slag, with soil-soluble compounds of suitable bases with phosphoric acid, from which latter, positive electrons only have been largely removed, and from which bases negative electrons have been largely removed, prior to the compounding thereof, the compounds having increased density and stability and diminished hygroscopicity.

53. A mixed granular fertilizer, comprising a slag, with soil-soluble compounds of phosphates and of potash, the latter having had negative electrons largely removed therefrom, and the former having had positive electrons largely removed therefrom, prior to the compounding thereof.

54. A product of values, comprising compounds of chemical reactions, of molecular associations, or of electrical adsorptions, of two suitable components of molecules, atoms or particles, solids, liquids or gases, from which components, there have been separately removed prior to the compounding thereof, heat-emitted electrons of one sign only, and opposites to each other, the compounds having increased density and stability.

55. A product of values, comprising compounds of chemical reactions, of molecular associations, or of electrical adsorptions compounded of two suitable components

- consisting of atoms or molecules or particles, solid or liquid or gaseous, from one of which components, there has been removed, prior to the compounding, heat-emitted electrons of one sign only, and the compounds having increased density and stability.
56. A product of values, including a fertilizer, comprising compounds of chemical reaction, of molecular associations or of electrical absorptions, compounded of two suitable components, whereof one component has duly taken up and combined with heat-emitted electrons prior to the compounding, and the compounds having increased density and stability and diminished hygroscopicity.
57. A product of values, including a fertilizer comprising compounds of two suitable components, from one of which components there has been removed prior to the compounding, heat-emitted electrons of one sign only, and to the other of which components, there have been added and combined therewith prior to the compounding, heat-emitted electrons of such latter sign, and the compounds having increased density and stability and diminished hygroscopicity.
58. A product of values, including a fertilizer, comprising compounds of two suitable components which have been separately oppositely electrified by heat, prior to and during the compounding, and the compounds having increased density and stability.
59. A product of values, including a fertilizer, comprising compounds of two suitable components, one of which has been electrified by heat, prior to and during the compounding, the compounds having increased density and stability.
60. A mixed fertilizer, in pulverized form, comprising a slag with soil-soluble basic phosphate compounds of molecules electrically compounded and having increased density and diminished hygroscopicity and increased stability, as compared to the like fertilizers not electrically compounded; and without soil-soluble ingredients detrimental as or with fertilizer components;

and from at least one of the components of which fertilizer there have been removed or earthed prior to or during the compounding, sundry electrons of one sign only.

61. A mixed fertilizer in granular form, comprising a metallurgical slag, with soil-soluble calcium phosphate and magnesium phosphate electrically compounded molecules, having increased density and diminished hygroscopicity, with increased stability; and from at least one of the components of which fertilizer there have been removed or earthed prior to or during the compounding, sundry electrons of one sign only.

62. A sulfate of ammonium compounded and recovered from a mixture of positively electrified insulated sulfur gases with negatively electrified insulated ammonia gases; such electrifications being attained by the earthing therefrom, separately of the opposite electrons of heat emissions, prior to the compounding; the compound having increased density and stability and diminished hygroscopicity.

63. In an apparatus as described, a hollow rabble stirrer, of conductor material, with insulator handle, with means of passing cooling fluids through the hollows thereof.

64. In an apparatus as described, supports of insulator dielectric refractory material, with perforations therethrough, with means of cooling the supports with cold air or waters or the like circulating through the perforations.

65. In an apparatus as described, a hollow cylindrical rabble stirrer, of conductor material, with insulator handle, with means of passing gases or powders or the like therethrough, into the materials being stirred.

In testimony whereof, I have hereto affixed my hand and seal in the presence of two witnesses.

JACOB E. BLOOM. [L. s.]

Witnesses:

EMMA BLOOM,  
ERWIN M. RIEBE.